

June 18, 1963

A. RIZO-PATRÓN R

3,094,484

PROCESS OF FROTH FLOTATION OF ORES

Filed Aug. 22, 1958

17 Sheets-Sheet 1

FIG. 1



FIG. 1a

| TEST<br>N <sup>o</sup> | pH<br>(1) | ΔΦ<br>(2) | TEST<br>N <sup>o</sup> | pH   | ΔΦ    | TEST<br>N <sup>o</sup> | pH   | ΔΦ    | TEST<br>N <sup>o</sup> | pH   | ΔΦ    |
|------------------------|-----------|-----------|------------------------|------|-------|------------------------|------|-------|------------------------|------|-------|
| 24                     | 7.30      | -0.66     | 33                     | 9.24 | +3.38 | 45                     | 9.45 | +2.54 | 69                     | 9.60 | +0.90 |
| 25                     | 7.60      | -1.06     | 34                     | 9.35 | +2.35 | 46                     | 9.43 | +2.58 | 70                     | 9.50 | +0.83 |
| 26                     | 7.90      | -1.18     | 35                     | 9.52 | +2.52 | 47                     | 9.43 | +2.40 | 71                     | 9.30 | +3.50 |
| 27                     | 8.25      | -0.43     | 36                     | 9.81 | -0.75 | 48                     | 9.52 | +2.02 | 72                     | 8.97 | +3.05 |
| 28                     | 8.52      | +0.51     | 37                     | 9.73 | +0.45 | 49                     | 9.64 | +0.67 |                        |      |       |
| 29                     | 8.87      | +2.70     | 40                     | 9.05 | +2.23 | 50                     | 9.39 | +2.70 |                        |      |       |
| 30                     | 9.00      | +3.46     | 42                     | 9.27 | +3.78 | 66                     | 9.15 | +2.25 |                        |      |       |
| 31                     | 9.18      | +3.66     | 43                     | 9.32 | +3.07 | 67                     | 8.82 | +1.80 |                        |      |       |
| 32                     | 9.15      | +3.39     | 44                     | 9.36 | +2.83 | 68                     | 8.12 | -2.79 |                        |      |       |

(2) ΔΦ in  
% minutes<sup>-1</sup>

Example 1

High grade oxidized  
lead ore from Pichita

Conditions of Tests

Grind:

Dilution = ± 60% solids

Ore weight = 1200 gr

Time = 4 minutes

Fineness = 100% - 48 mesh

Flotation: (1/32 split portions)

Dilution (P<sub>s</sub>) = ± 20% solids

Conditioning = ± 1/2 minutes

Time : as required

Results:

Equal differential floatability curves plotted.

$$\Delta\Phi = \frac{w}{t} \left[ \frac{f - (m-f)}{h - (m-h)} \right]$$

w = % weight of concentrate

t = flotation time in minutes

f = Pb grade of concentrate

h = Pb grade of heads (31%)

m = Pb grade of cerussite (77.5%)

Predetermined Basic  
Conditions for Plant  
Operational Control

Pulp density:

$$d_p = \frac{d_o \cdot 100}{P_s + d_o (100 - P_s)}$$

d<sub>o</sub> = specific gravity of ore = 3.20

$$\therefore d_p = 1.17$$

Reagents:

$$\text{Ratio NaSil.} = \frac{22}{3} = 7\frac{1}{3}$$

Resultant pH = ± 9.15

(to be reached and maintained in the plant thru the controlled addition of the proportioned reagent(s))

INVENTOR.

Alfonso Rizo-Patrón R  
BY *Byrly, Townsend,  
Watson & Churchill  
Atty's.*

June 18, 1963

A. RIZO-PATRÓN R

3,094,484

PROCESS OF FROTH FLOTATION OF ORES

Filed Aug. 22, 1958

17 Sheets-Sheet 2

FIG. 2



Example 1

Oxidized lead ore from Pichita

Conditions of Tests

Grind:

2 batches of dry ore  
Ore weight: 500 gr. per batch  
Time: 10 minutes per batch  
Fineness: 100% -48 mesh.

Flootation

Dilution ( $P_3$ ): 17.6% Solids  
Weight of ore per test: 50 gr.  
Conditioning:  $\pm 1\frac{1}{2}$  minutes.  
Time: as required by each test.

Results

Equal differential floatability curves plotted.

$$\Delta\phi = \frac{w}{t} \left[ \frac{f}{h} - \frac{(m-f)}{(m-h)} \right]$$

$w$  = % Weight of concentrate  
 $t$  = Flotation time in minutes  
 $f$  = Pb grade of concentrate  
 $h$  = Pb grade of heads ( $\pm 21\%$ )  
 $m$  = Pb grade of cerussite (77.5%)



SECTION A-A'

| Test No. | pH   | $\Delta\phi$ (1) | Test No. | pH   | $\Delta\phi$ (1) |
|----------|------|------------------|----------|------|------------------|
| 83       | 7.40 | -0.69            | 94       | 8.30 | +1.54            |
| 84       | 7.70 | -0.45            | 95       | 8.83 | +5.63            |
| 85       | 8.40 | +0.56            | 96       | 7.30 | -0.85            |
| 86       | 8.85 | +2.41            | 97       | 9.52 | +2.20            |
| 87       | 9.15 | +2.57            | 98       | 8.82 | +4.61            |
| 88       | 8.72 | +3.14            | 99       | 8.63 | +3.64            |
| 89       | 9.07 | +5.10            | 100      | 9.00 | +4.20            |
| 90       | 9.05 | +5.33            | 101      | 8.90 | +4.67            |
| 91       | 9.32 | +3.46            | 123      | 9.22 | +4.64            |
| 92       | 9.60 | +2.74            |          |      |                  |
| 93       | 9.21 | +4.16            |          |      |                  |

(1) in % minutes<sup>-1</sup>

$$\text{Pulp density: } d_p = \frac{d_0 \times 100}{P_3 + d_0 (100 - P_3)}$$

$$P_3 = 17.6\% \quad d_0 = 3.15 \text{ (specific gravity of ore)}$$

$$\therefore d_p = 1.14$$

$$\text{Reagents: } \frac{\text{NaSil}}{\text{R-710}} = \frac{23}{1.3} = 17.7$$

Resultant pH:  $\pm 8.90$

(to be reached and maintained in the plant thru the controlled addition of the proportioned reagents).

INVENTOR.

Alfonso Rizo-Patrón R.

BY Byerly, Townsend,  
Watson & Churchill  
Atty's

June 18, 1963

A. RIZO-PATRÓN R

3,094,484

## PROCESS OF FROTH FLOTATION OF ORES

Filed Aug. 22, 1958

17 Sheets-Sheet 3

TABLE NO. I-A Flotation 24-26-31  
 TEST NO. 36-48-72 INVESTIGATION NO. 1  
 CONDITIONS AND REAGENTS PROBLEM NO. Example 1  
 Pichita Ore: Pb: ± 30%.

| POINT OF ADDITION | CONDITIONS |                       |      | REAGENTS POUNDS PER TON. |           |          |           |              |         | OBSERVATIONS DURING TEST |                                                           |
|-------------------|------------|-----------------------|------|--------------------------|-----------|----------|-----------|--------------|---------|--------------------------|-----------------------------------------------------------|
|                   | TIME MIN.  | % <sub>o</sub> SOLIDS | pH   | NaSiI 3.9                | R-710 10% | R-710 5% | R-710 3.9 | NaSiI 33° Be | Ore 9t. | H <sub>2</sub> O cc      |                                                           |
| Grinding          | 4          | ± 60                  | Nat. | drops                    | drops     | cc       | —         | —            | 1,200   | 600                      | -48 mesh pulp split wet into 32 portions.                 |
| Test 24           | 6          |                       | 7.30 | —                        | —         | 1        | 2.19      | —            |         |                          | Bad conditions; very bulky, big bubbly froth.             |
| " 26              | 6          |                       | 7.90 | 2                        |           | 1        | 2.05      | 6.15         |         |                          | Somewhat better looking froth, but still very big bubbles |
| " 31              | 6          |                       | 9.18 | 7                        |           | 1        | 2.26      | 23.75        |         |                          | Excellent selective flotn. not very abundant.             |
| " 36              | 6          |                       | 9.81 | 16                       |           | 1        | 2.04      | 48.9         |         |                          | Almost nil, bad flotn. overflow of scum like froth.       |
| " 48              | 6          |                       | 9.52 | 13                       | 51        |          | 5.83      | 38.0         |         |                          | Rapid and persistent, loaded froth flotation.             |
| " 72              | 8          |                       | 9.10 | 7                        | 56        |          | 5.93      | 17.6         |         |                          | Good conditions, persistent flotn.                        |

REMARKS: 1 drop of NaSiI 3.9 = 2.79 lb/ton on 50 grams ore basis.  
 17 drops of R-710 (10%) = 2 lbs/ton on 50 gr. ore basis.

## METALLURGICAL RESULTS

| PRODUCT | WEIGHT |                | ASSAYS     | ΔΦ       | Pb CONTENT IN 100 PARTS H | DISTRIBUTIONS    |                     |                       | E <sub>m</sub><br>%                                  |
|---------|--------|----------------|------------|----------|---------------------------|------------------|---------------------|-----------------------|------------------------------------------------------|
|         | GRAMS  | % <sub>o</sub> |            |          |                           | Pb% <sub>o</sub> | % min <sup>-1</sup> | Pb                    |                                                      |
| F-24    | 8.6    | 18.8           | f = 29.5   | -0.66    | 5.55                      | 7.15             | 11.65               | 16.55 - 20.50 = -3.95 |                                                      |
| S-24    | 37.0   | 81.2           | s = 34.4   |          | 27.93                     | 36.0             | 45.2                | 63.45                 | -3.95                                                |
| H-24    | 45.6   | 100.0          | h = (33.5) |          | 33.48                     | 43.15            | 56.85               | 100.00                |                                                      |
| F-26    | 7.9    | 16.3           |            | 27.0     | -1.18                     | 4.40             | 5.68                | 10.62                 | 12.5 - 19.55 = -7.05                                 |
| S-26    | 41.0   | 83.7           |            | 37.0     |                           | 30.97            | 39.8                | 43.90                 | 87.5                                                 |
| H-26    | 48.9   | 100.0          |            | (35.37)  |                           | 35.37            | 45.48               | 54.52                 | 100.0                                                |
| F-31    | 17.0   | 38.5           |            | 45.0     | +3.66                     | 17.325           | 22.40               | 16.10                 | 50.8 - 28.8 = 22.0                                   |
| S-31    | 27.2   | 61.5           |            | 27.3     |                           | 16.789           | 21.60               | 39.90                 | 49.2                                                 |
| H-31    | 44.2   | 100.0          |            | (34.114) |                           | 34.114           | 44.0                | 56.0                  | 100.0                                                |
| F-36    | 6.1    | 12.4           |            | 26.3     | -0.75                     | 3.26             | 4.20                | 8.2                   | 9.8 - 14.3 = -4.5                                    |
| S-36    | 43.0   | 87.6           |            | 34.1     |                           | 29.87            | 38.50               | 49.1                  | 90.2                                                 |
| H-36    | 49.1   | 100.0          |            | (33.13)  |                           | 33.13            | 42.70               | 57.3                  | 100.0                                                |
| F-48    | 25.7   | 46.1           |            | 39.1     | +2.01                     | 18.0             | 23.2                | 22.9                  | 53.0 - 40.9 = 12.1                                   |
| S-48    | 30.2   | 53.9           |            | 29.8     |                           | 16.0             | 20.6                | 33.3                  |                                                      |
| H-48    | 55.9   | 100.0          |            | (34.0)   |                           | 34.0             | 43.8                | 56.2                  |                                                      |
| F-72    | 34.7   | 62.3           |            | 36.9     | +3.05                     | 23.0             |                     |                       | R <sub>m</sub> F - R <sub>g</sub> F = E <sub>m</sub> |
| S-72    | 21.0   | 37.7           |            | 17.7     |                           | 6.7              |                     |                       | 77.4 - 53.0 = 24.4                                   |
| H-72    | 55.7   | 100.0          |            | (29.7)   |                           | 29.7             |                     |                       | +24.4                                                |

$$\text{RATIO OF CONCENTRATION: } K = \frac{f-s}{h-s} \quad \Delta\Phi = \frac{E_m}{t}$$

REMARKS:

$$E_m = \frac{h-s}{f-s} \left[ \frac{f}{h} - \frac{m-f}{m-s} \right]$$

$$m = 77.5\% \text{ Pb (cerussite)}$$

## INVENTOR.

Alfonso Rizo-Patrón R.  
 BY  
 Bixby, Townsend, Watson & Churchill  
 Attn: J.

June 18, 1963

A. RIZO-PATRÓN R

3,094,484

## PROCESS OF FROTH FLOTATION OF ORES

Filed Aug. 22, 1958

17 Sheets-Sheet 4

TABLE NO. I-B Flotation TEST NO. 66 INVESTIGATION NO. 1  
CONDITIONS AND REAGENTS PROBLEM NO. Example 1  
Pichita Ore: Pb: ±30%.

| POINT OF ADDITION               | CONDITIONS    |             |      | REAGENTS POUNDS PER TON. |                    |  |                  | OBSERVATIONS DURING TEST |                                             |
|---------------------------------|---------------|-------------|------|--------------------------|--------------------|--|------------------|--------------------------|---------------------------------------------|
|                                 | TIME<br>MINS. | %<br>SOLIDS | PH   | Na<br>Sili.              | R-<br>710<br>(3.3) |  | Humid<br>Ore gr. | H <sub>2</sub> O<br>cc   |                                             |
| Grinding                        | 4             | ±60         | Nat. |                          |                    |  | 1,200            | 600                      | 100% - 48 mesh; wet split into 32 portions. |
| Conditioning                    | 1 1/2         | (21)        | 9.15 | 28.5                     | 9.5                |  |                  |                          | 1/32 portion of wet split pulp.             |
| Rougher                         | 10            | (21)        | -    |                          |                    |  |                  |                          | Very abundant silky flotation.              |
| Cleaner<br>(2 stages)<br>(each) | ± 7           | (±7.5)      | -    | No additions             |                    |  |                  |                          | Good, selective conditions.                 |
| Re-cleaner<br>(1 stage)         | 5             | (±11)       | -    | No additions             |                    |  |                  |                          | Excellent, very selective conditions.       |

REMARKS: Specific gravity of ore = ± 3.2 ∴ Percent solids (for rougher pulp):  
 Volume of flotation pulp = 250 cc.  $P_3 = \frac{61.3}{61.3 + (250 - \frac{61.3}{3.2})} = \frac{61.3}{292.1} = 21\%$

$P_S = 21\%$  solids by weight.

## METALLURGICAL RESULTS

| PRODUCT             | WEIGHT |         | ASSAYS |        |        | Pb CONTENT IN 100 PARTS H |            |        | DISTRIBUTIONS |         |        | Em<br>% |  |
|---------------------|--------|---------|--------|--------|--------|---------------------------|------------|--------|---------------|---------|--------|---------|--|
|                     | GRAMS  | %       | Pb%    | Pb%    | Pb%    | Rougher                   | Re-cleaner | Final  | Pb%           | Rougher | Final  | Gangue  |  |
| F <sub>RC</sub> -66 | 18.4   | 30.0    |        | 59.3   | 59.3   |                           | 17.8       | 17.8   |               | 61.8    | (11.2) | 50.6    |  |
| M-66                | 23.5   | 38.3    |        | 15.6   |        |                           | 6.0        |        |               |         |        |         |  |
| F-66                | 41.9   | 68.3    | 34.9   |        |        | 23.8                      |            |        | 82.9          |         | (60.3) | 22.6    |  |
| S-66                | 19.4   | 31.7    | 15.7   |        |        | 5.0                       | (5.0)      |        | 17.1          |         |        |         |  |
| M+S-66              | (42.9) | (70.0)  |        | (15.7) |        |                           |            | (11.0) |               | 38.2    |        |         |  |
| H-66                | (61.3) | (100.0) | (28.8) | (28.8) | (28.8) | (28.8)                    | (28.8)     | (28.8) | 100.0         | 100.0   |        |         |  |

RATIO OF CONCENTRATION: 3.33 : 1

In this test the cleaner and re-cleaner

REMARKS: (slide rule calculations) tailings were mixed and called M-66.

Since these middlings assayed less than the rougher tailings, they were assigned totally to the tailings in the final distribution of values.

$$Em \text{ (rougher)} = 0.683 \left[ \frac{34.9}{28.8} - \frac{77.5 - 34.9}{77.5 - 28.8} \right] = 22.6\%$$

$$Em \text{ (final)} = \frac{28.8 - 15.7}{59.3 - 15.7} \left[ \frac{59.3}{28.8} - \frac{77.5 - 59.3}{77.5 - 28.8} \right] = 50.6\%$$

Figures in parenthesis are values calculated from the experimental data actually obtained.

$$\Delta \Phi \text{ (rougher)} = 2.26 \text{ min}^{-1} \times \%$$

## INVENTOR.

Alfonso Rizo-Patrón R.

BY  
 Blyle, Townsend, Watson & Churchill  
 A.H.P.

June 18, 1963

A. RIZO-PATRÓN R

3,094,484

PROCESS OF FROTH FLOTATION OF ORES

Filed Aug. 22, 1958

17 Sheets-Sheet 5

TABLE NO. I-C

Flotation 84-88-90  
TEST NO. 91-94-97

INVESTIGATION NO. 2

PROBLEM NO. Example 1

Pichita Ore :  $\pm 20\% \text{ Pb}$ .

| POINT OF ADDITION | CONDITIONS    |             |      | REAGENTS POUNDS PER TON. |              |               | Weight | OBSERVATIONS DURING TEST |            |
|-------------------|---------------|-------------|------|--------------------------|--------------|---------------|--------|--------------------------|------------|
|                   | TIME<br>MINS. | %<br>SOLIDS | PH   | Nas1.<br>3.22            | R-710<br>10% | Nas1/<br>3.22 | R-710  | Em                       | Ore<br>gr. |
| Grinding          | 10            | 100         | —    | drops                    | drops        |               |        | %                        | 500        |
| Test 84           | 12 1/2        | (17.6)      | 7.70 | 2                        | 25           |               | 4.24   | 3.12                     | -5.6       |
| " 88              | 8             | "           | 8.72 | 13                       | 22           |               | 27.8   | 2.77                     | +25.1      |
| " 90              | 6             | "           | 9.05 | 13                       | 13           |               | 27.9   | 1.64                     | +32.0      |
| " 91              | 9             | "           | 9.32 | 16                       | 17           |               | 34.8   | 2.18                     | +31.3      |
| " 94              | 8             | "           | 8.30 | 5                        | 17           |               | 10.7   | 2.14                     | +12.3      |
| " 97              | 6             | "           | 9.52 | 20                       | 8            |               | 42.1   | 0.99                     | +13.2      |

REMARKS: Specific gravity of ground ore = 3.15

Volume of flotation pulp in each test = 250 cc.

Percent solids by weight  $P_s = \frac{50}{50 + (250 - \frac{50}{3.15})} = \frac{50}{284.1} = 17.6\%$

METALLURGICAL RESULTS

| PRODUCT | WEIGHT |         | ASSAYS | Pb CONTENT IN 100 PARTS H | DISTRIBUTIONS | $\Delta\Phi$ | Em    |
|---------|--------|---------|--------|---------------------------|---------------|--------------|-------|
|         | GRAMS  | %<br>as |        |                           |               |              |       |
| F-84    | 22.6   | 46.5    | 19.9   | 9.20                      | 42.3          | -0.45        |       |
| S-84    | 24.6   | 53.5    | 23.5   | 12.60                     |               |              | -5.6  |
| H-84    | 47.2   | 100.0   |        | (21.8)                    |               |              |       |
| F-88    | 25.0   | 53.5    | 29.3   | 15.6                      | 71.4          | +3.14        |       |
| S-88    | 21.8   | 46.5    | 13.6   | 6.3                       |               |              | +25.1 |
| H-88    | 46.8   | 100.0   |        | (21.9)                    |               |              |       |
| F-90    | 20.3   | 43.4    | 33.9   | 14.65                     | 65.8          | +5.33        |       |
| S-90    | 26.4   | 56.6    | 13.6   | 7.70                      |               |              | +32.0 |
| H-90    | 46.7   | 100.0   |        | (22.35)                   |               |              |       |
| F-91    | 20.5   | 44.6    | 33.0   | 14.75                     | 67.2          | +3.46        |       |
| S-91    | 25.5   | 55.4    | 13.0   | 7.2                       |               |              | +31.3 |
| H-91    | 46.0   | 100.0   |        | (21.95)                   |               |              |       |
| F-94    | 19.3   | 41.1    | 25.5   | 10.5                      | 50.2          | +1.54        |       |
| S-94    | 27.6   | 58.9    | 17.7   | 10.4                      |               |              | +12.3 |
| H-94    | 46.9   | 100.0   |        | (20.9)                    |               |              |       |
| F-97    | 4.0    | 8.4     | 47.9   | 4.0                       | 17.8          | +2.2         |       |
| S-97    | 43.5   | 91.6    | 20.2   | 18.5                      |               |              | +13.2 |
| H-97    | 47.5   | 100.0   |        | (22.5)                    |               |              |       |

RATIO OF CONCENTRATION:  $K = \frac{f}{w}$

REMARKS: Assays of heads calculated from weights and assays of products of each test.

$$E_m = w \left[ \frac{f}{h} - \frac{m-f}{m-h} \right] \quad \Delta\Phi = \frac{E_m}{t}$$

$m = 77.5\% \text{ Pb}$  (cerussite).

INVENTOR.

Alfonso Rizo-Patrón R.

BY  
Byers, Townsend, Watson & Churchill  
Attn: S

June 18, 1963

A. RIZO-PATRÓN R

3,094,484

## PROCESS OF FROTH FLOTATION OF ORES

Filed Aug. 22, 1958

17 Sheets-Sheet 6

| TABLE NO. <u>I-D</u> |               |                      | Flotation                                    |                 |       |    | INVESTIGATION NO. <u>2</u>         |      |     |
|----------------------|---------------|----------------------|----------------------------------------------|-----------------|-------|----|------------------------------------|------|-----|
|                      |               |                      | TESTING NO. <u>124-123</u>                   |                 |       |    | PROBLEM NO. <u>Example 1</u>       |      |     |
|                      |               |                      | CONDITIONS AND REAGENTS                      |                 |       |    | Pichita Ore: $\pm 20\% \text{ Pb}$ |      |     |
| POINT OF ADDITION    | TIME<br>MINS. | CONDITIONS<br>SOLIDS | REAGENTS                                     | POUNDS PER TON. |       |    |                                    |      |     |
|                      |               |                      | NaSi <sub>1.322</sub><br>R-710<br>3.22-G 10% | cc              | drops |    |                                    |      |     |
| Grinding             | 10            | 100                  | —                                            | —               | —     |    |                                    |      |     |
| Conditioning         | 1½            | 17.6                 | 8.85                                         | —               | 6     | —  | 24.5                               | 1.63 |     |
| Rougher              | 7             |                      | 9.22                                         | 5               | —     | —  | 10.2                               |      | 124 |
| Cleaner              | 5             |                      |                                              | 1               | —     | —  | 2.04                               |      | " " |
| Re-cleaner           | 2½            |                      |                                              | No additions    |       |    |                                    |      | " " |
| Grinding             | 10            | 100                  | —                                            | —               | —     | —  |                                    |      |     |
| Conditioning         | 1½            | 17.6                 | 9.22                                         | 14              | —     | 14 | 30                                 | 1.77 | 123 |
| Rougher              | 7             |                      | 9.22                                         | —               | —     | —  |                                    |      |     |
| Scavenger            | 5             |                      | 9.22                                         | 2               | —     | 8  | 17.2                               | 1.01 |     |

REMARKS: Vanning 5-123 practically no cerussite concentrate was obtained.  
1 drop of NaSi<sub>1.322</sub> = 2.0 lbs/ton on 50 gr. ore basis.

| PRODUCT                | WEIGHT |        | ASSAYS      |        |           | Pb CONTENT IN 100 PARTS H |            | DISTRIBUTIONS |               |        | Em (%)               |       |
|------------------------|--------|--------|-------------|--------|-----------|---------------------------|------------|---------------|---------------|--------|----------------------|-------|
|                        | GRAMS  | %      | Pb%         | Pb%    | Pb%       | Rougher                   | Re-cleaner | Final         | % Pb          | % Pb   | Final                |       |
|                        |        |        | Rougher     | Final  | Scavenger | Fe + F <sub>s</sub>       | Rougher    | Final         | Rougher       | Final  | Rougher              |       |
| FRC-124                | 10.3   | 21.1   | 62.4 (33.7) | (62.4) | (18.85)   | 13.25                     | (15.4)     | 79.4 (65.0)   | +58.5         |        |                      |       |
| MRC-124                | 5.1    | 10.4   | 17.8        |        |           |                           | 1.85       |               |               |        |                      | +33.5 |
| Mc-124                 | 12.0   | 24.5   | 15.3        |        |           |                           | 3.75       |               |               |        |                      |       |
| S-124                  | 21.5   | 44.0   | 11.1        | 11.1   | (11.1)    | 4.89                      | 4.89       | (8.3)         | 20.6 (35.0)   |        |                      |       |
| H-124                  | 48.9   | 100.0  | (23.74)     |        |           | (23.74)                   | 23.74      | (23.7)        | 100.0 (100.0) |        |                      |       |
| FR-123                 | 21.7   | 46.5   | 31.5        | 31.5   |           | 14.60                     | 14.60      |               | 70.0          |        |                      | +32.5 |
| SR-123                 | (25.0) | (53.5) | (11.75)     | 11.75  |           | (6.27)                    |            |               | 30.0          |        |                      |       |
| F <sub>3</sub> -123    | 7.0    | 15.0   | 15.6        |        |           |                           | 2.34       |               |               |        |                      |       |
| FR+F <sub>3</sub> -123 | (28.7) | (61.5) | (27.5)      |        | (27.5)    |                           | (16.94)    |               | 81.0          | +26.75 |                      |       |
| S <sub>3</sub> -123    | 18.0   | 38.5   | 10.2        |        | 10.2      |                           | 3.93       | 3.93          |               | 19.0   |                      |       |
| H-123                  | 46.7   | 100.0  |             |        |           | (20.87)                   | (20.87)    | (20.87)       | 100.0         | 100.0  | Rougher<br>Scavenger |       |

$$\text{RATIO OF CONCENTRATION: } K_{124} = \frac{62.4 - 11.1}{23.74 - 11.1} = \frac{51.3}{12.64} = 4.05 \quad \therefore \omega = \frac{1}{K} = \frac{1}{4.05} = 24.7\% \text{ (final)}$$

m = 77.5% Pb (cerussite)

Test 124:

$$Em(\text{rougher}) = 0.56 \left[ \frac{33.7}{23.74} - \frac{77.5 - 33.7}{77.5 - 23.74} \right] = +33.5\%$$

$$\Delta \Phi(\text{rougher 124}) = +4.78 \text{ min}^{-1} \times \%$$

$$Em(\text{final}) = 0.247 \left[ \frac{62.4}{23.74} - \frac{77.5 - 62.4}{77.5 - 23.74} \right] = +58.5\%$$

Test 123:

$$Em(\text{rougher}) = 0.465 \left[ \frac{31.5}{20.87} - \frac{77.5 - 31.5}{77.5 - 20.87} \right] = +32.5\%$$

$$Em(\text{scavenger}) = 0.615 \left[ \frac{27.5}{20.87} - \frac{77.5 - 27.5}{77.5 - 20.87} \right] = +26.75\% \quad \text{BY} \quad \text{Alfonso Rizo-Patrón R.}$$

$$\Delta \Phi(\text{rougher}) = +4.65 \text{ min}^{-1} \times \%; \Delta \Phi(\text{scavenger}) = +2.23 \text{ min}^{-1} \times \%$$

INVENTOR.

Alfonso Rizo-Patrón R.  
By  
Byrd, Townsend, Watson & Gresham

Attn's

June 18, 1963

A. RIZO-PATRÓN R

3,094,484

## PROCESS OF FROTH FLOTATION OF ORES

Filed Aug. 22, 1958

17 Sheets-Sheet 7

TABLE NO. I-E Flotation and tails' tabling TEST NO. 131  
 INVESTIGATION NO. 2  
 PROBLEM NO. Example 1  
Pichita Ore: ± 20% Pb.

| POINT OF ADDITION | CONDITIONS    |             |      | REAGENTS POUNDS PER TON.       |                       |           | OBSERVATIONS DURING TEST |                                          |
|-------------------|---------------|-------------|------|--------------------------------|-----------------------|-----------|--------------------------|------------------------------------------|
|                   | TIME<br>MINS. | %<br>SOLIDS | PH   | 3.32/708<br>R.H.R. 15<br>10.26 | NaS1<br>3.22<br>10.26 | R-708     |                          |                                          |
| Grinding          | 6             | 45          | Nat. | cc                             | cc                    |           | 800 1,200                | 100% -65 mesh                            |
| Conditioning      | 1 1/2         | 20          | 7.43 | 135                            | —                     | 32.5 2.16 |                          |                                          |
| Rougher           | 18            |             | 9.25 |                                |                       |           |                          | Good abundant but dark & slow flotation. |
| Cleaner           | 9             |             |      | No additions                   |                       |           |                          | Good but dark fltn.                      |
| Re-cleaner        | 9             |             |      | —                              | 10                    | 2.4       | —                        | Good, still dark fltn.                   |
|                   |               |             |      |                                |                       |           |                          |                                          |
|                   |               |             |      |                                |                       |           |                          | + Total reagents.                        |
|                   |               |             |      |                                |                       |           |                          |                                          |

REMARKS: Water available at the Pichita plant used in test.

Flotation tailings passed through Wilfley concentrating table, and a fairly abundant light colored concentrate was obtained (c-131).

Test made in the metallurgical laboratory of the Pichita mine.

## METALLURGICAL RESULTS

| PRODUCT     | WEIGHT  |        | ASSAYS  |         |         | Pb CONTENT IN 100 PARTS/H |         | DISTRIBUTIONS |                 |               | Em<br>%     |         |
|-------------|---------|--------|---------|---------|---------|---------------------------|---------|---------------|-----------------|---------------|-------------|---------|
|             | GRAMS   | %      | Pb %    | Pb %    | Pb %    | All products              | Rougher | Final         | % Pb<br>Rougher | % Pb<br>Final | %<br>Gangue |         |
| H - 131     | 835.2   | 100.0  | (18.66) | (18.66) | (18.66) | (18.66)                   | (18.66) | (18.66)       | 100.0           | 100.0         |             | Final:  |
| FRC - 131   | 160.9   | 19.3   | 59.8    |         | 59.8    | 11.60                     |         | 15.23         |                 | 81.6          | 7.7         | +73.9   |
| MRC - 131   | 45.0    | 5.4    | 25.3    | (37.7)  |         | 1.37                      | (14.32) |               | 76.8            |               | 25.7        | +51.1   |
| Mc - 131    | 111.5   | 13.3   | 10.1    |         |         | 1.35                      |         |               |                 |               |             | Rougher |
| S - 131     | 517.8   | 62.0   | 7.0     | 7.0     |         | 4.34                      | 4.34    |               | 23.2            |               |             |         |
| S' - 131    | (489.7) | (62.0) | 7.0     | (7.0)   |         | 4.34                      | (4.34)  |               |                 |               |             |         |
| C - 131     | 55.9    | 7.1    | 25.7    | 25.7    |         | 1.83                      | 1.83    |               |                 |               |             |         |
| M - 131     | 85.4    | 10.8   | 4.5     |         |         | 0.49                      |         |               |                 |               |             |         |
| T - 131     | 49.1    | 6.2    | 4.9     | (4.59)  |         | 0.30                      | 2.51    |               |                 |               |             |         |
| L - 131     | 155.7   | 19.7   | 6.6     |         |         | 1.30                      |         |               |                 |               |             |         |
| Lost slimes | (143.6) | 18.2   | (2.3)   |         |         | (0.42)                    |         |               |                 |               |             |         |
| Final tails |         |        |         |         |         | (4.59)                    |         | (3.43)        |                 | 18.4          |             |         |

RATIO OF CONCENTRATION:  $K_{131} = 59.8 - 4.59 / 18.66 - 4.59 = 3.93 \therefore w = \frac{1}{3.93} = 25.5\% \text{ (final)}$ REMARKS:  $S' = S (517.8 \text{ gr}) - \text{Sample separated for assay of S-131 (28.1 gr)} \therefore S' = 489.7 \text{ gr}$ 

$$Em = R_{Pb} F - R_g F$$

 $R_{Pb} F = \text{Recovery of lead in float} = w \cdot \frac{f}{h} \quad \& \quad R_g F = \text{Recovery of gangue in float} = w \cdot \frac{m-f}{m-h}$ 

$$\therefore Em \text{ (rougher)} = (0.38 \cdot \frac{37.7}{18.66}) - (0.38 \cdot \frac{77.5 - 37.7}{77.5 - 18.66}) = 76.8\% - 25.7\% = +51.1\%$$

$$Em \text{ (final)} = (0.255 \cdot \frac{59.8}{18.66}) - (0.255 \cdot \frac{77.5 - 59.8}{77.5 - 18.66}) = 81.6\% - 7.7\% = +73.9\%.$$

## INVENTOR.

Alfonso Rizo-Patrón R.

BY  
Byrly, Townsend, Watson, & Churchill

ATTY'S

Distribution of values made assuming that C-131 is reground and gives place to the same flotation separation as the one obtained with the original heads.  
 $\Delta \Phi \text{ (rougher)} = 2.84 \text{ min}^{-1} \cdot \%$

June 18, 1963

A. RIZO-PATRÓN R

3,094,484

## PROCESS OF FROTH FLOTATION OF ORES

Filed Aug. 22, 1958

17 Sheets-Sheet 8

TABLE NO. I-FFlotation TEST NO. "D"INVESTIGATION NO. 1  
PROBLEM NO. Example 1  
Pichita ore : ± 30% Pb.

| POINT OF ADDITION | CONDITIONS |          |      | REAGENTS POUNDS PER TON.    |            |       |                                   | OBSERVATIONS DURING TEST                                        |
|-------------------|------------|----------|------|-----------------------------|------------|-------|-----------------------------------|-----------------------------------------------------------------|
|                   | TIME MIN.  | % SOLIDS | PH   | 3.22/700 R-ARP 10% 15<br>cc | NaS1. 3.22 | R-708 | Humid ore gr. H <sub>2</sub> O cc |                                                                 |
| Grinding          | 33         | ± 42     | Nat. |                             |            |       | 1200 600                          | 100% - 100 mesh                                                 |
| Conditioning      | 1 1/2      |          |      | 160                         | 43.0       | 2.86  |                                   |                                                                 |
| Rougher           | 15         |          |      |                             |            |       |                                   | Good but slow flotation of dark froth.                          |
| Scavenger         | 5          |          |      | 40                          | 10.75      | 0.715 |                                   | Some more flotation                                             |
| Cleaner           | 10         |          |      | No additions                |            |       |                                   | More selective flotation                                        |
| Re-cleaner        | 10         |          |      | "                           | "          |       |                                   | Very selective lighter colored froth (liquid of pulp was dark). |
|                   |            |          |      |                             | 53.75      | 3.575 |                                   |                                                                 |

REMARKS: Test made in laboratory of the Pichita mine.

Vanning S-D gave a considerable amount of grayish Pb concentrate. Frc-D was almost pure cerussite.

Mrc &amp; Mc were combined and called M-D.

## METALLURGICAL RESULTS

| PRODUCT | WEIGHT  |        | Pb ASSAYS |         | Pb CONTENT IN 100 PARTS/H |          | % DISTRIBUTIONS |       |            | Em       |        |       |
|---------|---------|--------|-----------|---------|---------------------------|----------|-----------------|-------|------------|----------|--------|-------|
|         | GRAMS   | %      | Obtained  | Rougher | Final                     | Obtained | Rougher         | Final | Pb Rougher | Pb Final | Gangue | %     |
| Frc - D | 186.6   | 25.0   | 73.84     |         | 73.84                     | 18.4     |                 |       | 72.2       | 2.2      |        | +70.0 |
| M - D   | 160.0   | 21.4   | 27.25     |         |                           | 5.8      |                 |       |            |          |        |       |
| F - D   | (346.6) | (46.4) |           | (52.2)  |                           | (24.2)   |                 |       | 73.9       |          | 26.4   | +47.5 |
| S - D   | 400.0   | 53.6   | 16.20     | 16.20   | 16.20                     | 8.7      | 8.7             |       | 26.1       | 27.8     |        |       |
| H - D   | 746.6   | 100.0  |           | (32.9)  |                           | (32.9)   | (32.9)          |       |            |          |        |       |

$$\text{RATIO OF CONCENTRATION: } K = \frac{73.84 - 16.20}{32.90 - 16.20} = 3.09 \quad \therefore \quad W = \frac{1}{3.09} = 32.4\%$$

REMARKS: m = 77.5% Pb (cerussite)

$$E_m (\text{rougher}) = 0.464 \left[ \frac{52.2}{32.9} - \frac{77.5 - 52.2}{77.5 - 32.9} \right] = +47.5\%$$

$$E_m (\text{final}) = 0.324 \left[ \frac{73.84}{32.9} - \frac{77.5 - 73.84}{77.5 - 32.9} \right] = +70.0\%$$

$$\Delta \Phi (\text{rougher}) = -\frac{47.5}{20 \text{ min}} = 2.375 \text{ min}^{-1}\%$$

INVENTOR.

Alfonso Rizo-Patrón R.

BY  
Byrly, Townsend, Watson & Churchill  
Attys.

June 18, 1963

A. RIZO-PATRÓN R

3,094,484

## PROCESS OF FROTH FLOTATION OF ORES

Filed Aug. 22, 1958

17 Sheets-Sheet 9

TABLE NO. II-AFlotation 55-56-66  
TEST NO. 67-70-71INVESTIGATION NO. 3  
PROBLEM NO. Example 2Cerro de Pasco ore:  $\pm 11\% Pb$ 

| POINT OF ADDITION | CONDITIONS    |             |      | REAGENTS POUNDS PER TON. |             |               |       |                         | OBSERVATIONS DURING TEST |                                                      |
|-------------------|---------------|-------------|------|--------------------------|-------------|---------------|-------|-------------------------|--------------------------|------------------------------------------------------|
|                   | TIME<br>MINS. | %<br>SOLIDS | PH   | Nasil.<br>3.9            | R-710<br>5% | Nasil.<br>3.9 | R-710 | $\Delta\Phi$            | $E_m$                    |                                                      |
| Grinding          | 10            | $\pm 60$    | Nat. | 10 drops                 | 10 drops    |               |       | min <sup>-1</sup><br>X% | %                        | 100% -48 mesh<br>Wet splitting                       |
| Test 55           | 5             |             | 8.78 | 4                        | 10          | 12.6          | 0.55  | +0.14                   | +0.7                     | Very scarce flotation;<br>almost no frothing.        |
| " 56              | 5             |             | 7.52 | 1                        | 20          | 3.07          | 1.06  | +0.6                    | +3.0                     | Abundant but bubbly<br>froth                         |
| " 66              | 5             |             | 8.80 | 4                        | 50          | 10.1          | 2.19  | +0.9                    | +54.3                    | Excellent flotation;<br>not much frothing.           |
| " 67              | 6             |             | 7.16 | —                        | 58          | —             | 2.85  | -0.15                   | -0.93                    | A mountain of bubbles!<br>no selectivity.            |
| " 70              | 6             |             | 9.35 | 6                        | 58          | 19.6          | 3.28  | +2.81                   | +16.9                    | Very selective flotation;<br>but almost no frothing. |
| " 71              | 6             |             | 8.52 | 3                        | 58          | 9.6           | 3.22  | +0.67                   | +52.0                    | Excellent flotation;<br>ideal frothing.              |

REMARKS: 10 drops of R-710 (5%)  $\approx 0.52$  lb/ton on 50 gr. ore basis.

## METALLURGICAL RESULTS

| PRODUCT | WEIGHT |       | % ASSAYS |  | CONTENT IN 100 PARTS H |  | DISTRIBUTIONS |        |         |
|---------|--------|-------|----------|--|------------------------|--|---------------|--------|---------|
|         | GRAMS  | %     | Pb       |  | Pb                     |  | Pb            | Gangue | $E_m\%$ |
| F-55    | 3.7    | 8.25  | 12.2     |  | 1.01                   |  | 8.7           | 8.0    | +0.7    |
| S-55    | 44.0   | 91.75 | 11.6     |  | 10.61                  |  |               |        |         |
| H-55    | (47.7) |       |          |  | (11.62)                |  |               |        |         |
| F-56    | 11.9   | 24.4  | 13.3     |  | 3.25                   |  | 26.8          | 23.8   | +3.0    |
| S-56    | 37.0   | 75.6  | 11.8     |  | 8.92                   |  |               |        |         |
| H-56    | (48.9) |       |          |  | (12.17)                |  |               |        |         |
| F-66    | 18.1   | 30.35 | 31.9     |  | 9.68                   |  | 76.0          | 22.7   | +54.3   |
| S-66    | 41.6   | 69.65 | 4.4      |  | 3.06                   |  |               |        |         |
| H-66    | (59.7) |       |          |  | (12.74)                |  |               |        |         |
| F-67    | 14.0   | 26.5  | 11.3     |  | 3.0                    |  | 25.2          | 26.13  | -0.93   |
| S-67    | 38.8   | 73.5  | 11.5     |  | 8.45                   |  |               |        |         |
| H-67    | (52.8) |       |          |  | (11.45)                |  |               |        |         |
| F-70    | 8.3    | 18.0  | 20.4     |  | 3.68                   |  | 32.1          | 15.2   | +16.9   |
| S-70    | 37.7   | 82.0  | 9.1      |  | 7.45                   |  |               |        |         |
| H-70    | (46.0) |       |          |  | (11.13)                |  |               |        |         |
| F-71    | 16.2   | 34.6  | 26.7     |  | 9.26                   |  | 76.2          | 24.2   | +52.0   |
| S-71    | 30.5   | 65.4  | 4.4      |  | 2.89                   |  |               |        |         |
| H-71    | 46.7   |       |          |  | 12.15                  |  |               |        |         |

## RATIO OF CONCENTRATION

REMARKS:  $\Delta\Phi = \frac{E_m}{t}$  in minutes<sup>-1</sup> %

## INVENTOR

Alfonso Rizo-Patrón R.

BY  
Byrd, Townsend, Watson & Churchill  
ATL's.

June 18, 1963

A. RIZO-PATRÓN R

3,094,484

PROCESS OF FROTH FLOTATION OF ORES

Filed Aug. 22, 1958

17 Sheets-Sheet 10

TABLE NO. II-B

Flotation 104-105-107  
TESTING NO. 129-111-112  
INVESTIGATION NO. 4  
PROBLEM NO. Example 2  
Cerro de Pasco ore:  $\pm 5\% \text{ Pb}$

| POINT OF ADDITION | CONDITIONS |          |      | REAGENTS POUNDS PER TON. |               |       |              |       |                   | OBSERVATIONS DURING TEST |                                              |
|-------------------|------------|----------|------|--------------------------|---------------|-------|--------------|-------|-------------------|--------------------------|----------------------------------------------|
|                   | TIME MINS. | % SOLIDS | pH   | NaSIL R-710<br>3.22 10%  | NaSIL<br>3.22 | R-710 | $\Delta\phi$ | $E_m$ |                   |                          |                                              |
| Grinding          | 15         | 100      |      | drops                    | drops         |       |              |       | $\text{min}^{-1}$ | $\%$                     |                                              |
| Test 104          | 5          |          | 9.15 | 10                       | 8             | 20    | 0.94         | +0.18 | +0.89             |                          | Almost nil dry froth flotation.              |
| " 105             | 7          |          | 9.25 | —                        | 17            | —     | 2.0          | +3.8  | +26.6             |                          | Abundant bubbly but loaded froth flotation   |
| " 107             | 5          |          | 8.05 | 4                        | 17            | 8     | 2.0          | +7.49 | +37.4             |                          | = Good flotation, but still a little bubbly. |
| " 109             | 4          |          | 9.00 | 8                        | 17            | 16    | 2.0          | +2.35 | +9.4              |                          | Brittle froth, scarce scum-like flotation.   |
| " 111             | 4          |          | 8.60 | 6                        | 26            | 12    | 3.05         | +9.15 | +36.6             |                          | Good rapid flotation.                        |
| " 112             | 5          |          | 9.35 | 10                       | 26            | 20    | 3.05         | +0.53 | +2.65             |                          | Scace scum-like flotation.                   |

REMARKS:

METALLURGICAL RESULTS

| PRODUCT | WEIGHT |       | % ASSAYS |  | CONTENT IN 100 PARTS H |  |  | DISTRIBUTIONS |        |         |
|---------|--------|-------|----------|--|------------------------|--|--|---------------|--------|---------|
|         | GRAMS  | %     | Pb       |  | Pb                     |  |  | Pb            | Gangue | $E_m$ % |
| F-104   | 0.6    | 1.2   | 7.9      |  | 0.095                  |  |  | 2.05          |        | +0.89   |
| S-104   | 48.8   | 98.8  | 4.6      |  | 4.55                   |  |  |               |        |         |
| H-104   | 49.4   |       |          |  | (4.645)                |  |  |               |        |         |
| F-105   | 13.0   | 26.3  | 9.7      |  | 2.54                   |  |  | 51.0          | 24.4   | +26.6   |
| S-105   | 36.5   | 73.7  | 3.3      |  | 2.43                   |  |  |               |        |         |
| H-105   | 49.5   |       |          |  | (4.91)                 |  |  |               |        |         |
| F-107   | 10.0   | 20.2  | 14.3     |  | 2.89                   |  |  | 53.8          | 15.4   | +37.4   |
| S-107   | 39.5   | 79.8  | 3.1      |  | 2.47                   |  |  |               |        |         |
| H-107   | 49.5   |       |          |  | (5.36)                 |  |  |               |        |         |
| F-109   | 3.4    | 6.95  | 12.2     |  | 0.85                   |  |  | 15.7          | 6.3    | +9.4    |
| S-109   | 45.5   | 93.05 | 4.9      |  | 4.55                   |  |  |               |        |         |
| H-109   | 48.9   |       |          |  | (5.40)                 |  |  |               |        |         |
| F-111   | 10.0   | 20.4  | 13.2     |  | 2.70                   |  |  | 54.7          | 18.1   | +36.6   |
| S-111   | 39.2   | 79.6  | 2.8      |  | 2.23                   |  |  |               |        |         |
| H-111   | 49.2   |       |          |  | (4.93)                 |  |  |               |        |         |
| F-112   | 3.1    | 6.3   | 8.3      |  | 0.52                   |  |  | 8.7           | 6.05   | +2.65   |
| S-112   | 46.3   | 93.7  | 5.8      |  | 5.42                   |  |  |               |        |         |
| H-112   | 49.4   |       |          |  | 5.94                   |  |  |               |        |         |

RATIO OF CONCENTRATION:

REMARKS:  $\Delta\phi = \frac{E_m}{t} = \frac{w}{t} \left[ \frac{f}{h} - \frac{m-f}{m-h} \right]$  in  $\text{min}^{-1} \times \%$

INVENTOR:

Alfonso Rizo-Patrón R.

BY  
Boggs, Townsend, Watson & Churchill  
Atty's

June 18, 1963

A. RIZO-PATRÓN R

3,094,484

## PROCESS OF FROTH FLOTATION OF ORES

Filed Aug. 22, 1958

17 Sheets-Sheet 11

TABLE No. II-CFlotation 116INVESTIGATION No. 4  
PROBLEM No. Example 2  
Cerro de Pasco ore:  $\pm 5\%$  Pb.

| POINT OF ADDITION | CONDITIONS |          |      | REAGENTS POUNDS PER TON. |           |           |              | OBSERVATIONS DURING TEST |                                                        |
|-------------------|------------|----------|------|--------------------------|-----------|-----------|--------------|--------------------------|--------------------------------------------------------|
|                   | TIME MINS. | % SOLIDS | PH   | NaSi/3.22                | R-710 10% | NaSi/3.22 | R-710 0.6 g. |                          |                                                        |
| Grinding          | 25         | 56.5     |      | deeps                    | cc        |           | 650          | 450                      | 100% - 65 mesh.                                        |
| Conditioning      | 1 1/2      |          | 7.88 | 52                       | 6         |           | 1.92         |                          |                                                        |
| Rougher           | 6          |          | 8.00 |                          | 13        | —         |              |                          | Excellent flotation; somewhat bubbly froth at the end. |
| Cleaner           | 3          |          | 8.03 | No additions             |           |           |              |                          | Very good, abundant, more selective froth.             |
| Re-cleaner        |            |          |      | "                        | "         |           |              |                          | Good, selective flotation.                             |

REMARKS: Test made in the San Isidro (Lima) laboratory of the "Cia. Minera Chanchamayo S.A."

## METALLURGICAL RESULTS

| PRODUCT | WEIGHT  |       | PB ASSAY % | PB CONTENT IN 100 PARTS/H | % DISTRIBUTIONS |         |       | Em %             |
|---------|---------|-------|------------|---------------------------|-----------------|---------|-------|------------------|
|         | GRAMS   | %     |            |                           | Actual          | Rougher | Final |                  |
| Frc-116 | 25.6    | 4.08  | 38.5       | (38.5)                    | 1.58            |         |       | 52.8 (3.5) +49.3 |
| Mrc-116 | 42.5    | 6.77  | 8.1        |                           | 0.55            |         |       |                  |
| Mc-116  | 114.0   | 18.10 | 4.5        |                           | 0.82            |         |       |                  |
| F-116   | (28.95) |       | (10.2)     |                           | (2.95)          |         | 64.3  | (26.8) +37.5     |
| S-116   | 447.3   | 71.05 | 2.3        | 2.3                       | 1.63            | 1.63    | 35.7  | 47.2             |
| H-116   | 629.4   |       |            |                           | (4.58)          | (4.58)  | 100.0 | 100.0            |

$$\text{RATIO OF CONCENTRATION: } K = \frac{38.5 - 2.3}{4.58 - 2.3} = 15.9 \quad \therefore \omega = \frac{1}{15.9} = 6.28\%$$

REMARKS:

 $m = 77.5\%$  (assumed as cerussite)

$$E_m (\text{rougher}) = 0.2895 \left[ \frac{10.2}{4.58} - \frac{77.5 - 10.2}{77.5 - 4.58} \right] = +37.5\%$$

$$E_m (\text{final}) = 0.0628 \left[ \frac{38.5}{4.58} - \frac{77.5 - 38.5}{77.5 - 4.58} \right] = +49.3\%$$

$$\Delta \Phi (\text{rougher}) = \frac{+37.5\%}{6 \text{ min.}} = +6.26 \text{ min}^{-1}\%$$

INVENTOR.

Alfonso Rizo-Patrón R.

BY  
Byerly, Townsend, Watson +  
Churchill Atlys

June 18, 1963

A. RIZO-PATRÓN R

3,094,484

## PROCESS OF FROTH FLOTATION OF ORES

Filed Aug. 22, 1958

17 Sheets-Sheet 12

| TABLE NO. II-D    |              |                       | Flotation TEST No. I      |                     |                        | INVESTIGATION NO. 5   |  |                                                            |
|-------------------|--------------|-----------------------|---------------------------|---------------------|------------------------|-----------------------|--|------------------------------------------------------------|
|                   |              |                       | CONDITIONS AND REAGENTS   |                     |                        | PROBLEM NO. Example 2 |  |                                                            |
| POINT OF ADDITION | TIME<br>MIN. | PER<br>CENT<br>SOLIDA | R-708<br>10%<br>10%<br>cc | Nasil.<br>10%<br>cc | Nasil.<br>3.9<br>R-708 |                       |  | Cerro de Pasco Ore: ± 26% Pb.                              |
| Grinding          | 30           | 50                    | Nat.                      |                     |                        |                       |  | 100% - 65 mesh to flotation laboratory Denver cell.        |
| Conditioning      | 1            |                       |                           | 150                 | 34                     | 3.4                   |  |                                                            |
| Rougher           | 14           |                       |                           |                     |                        |                       |  | Excellent flotation conditions.                            |
| Cleaner           | 7            |                       |                           | 10                  | 2                      |                       |  | Excellent, very selective flotation of almost white froth. |
|                   |              |                       |                           |                     |                        |                       |  |                                                            |
|                   |              |                       |                           |                     |                        |                       |  |                                                            |

REMARKS: Test made in the laboratory of the Pichita mine.

No re-cleaning was necessary with this ore.

| PRODUCT            | WEIGHT |        | Pb ASSAYS % |         |        | Pb CONTENT IN 100 PARTS H |         | DISTRIBUTIONS |       |        | Em<br>% |
|--------------------|--------|--------|-------------|---------|--------|---------------------------|---------|---------------|-------|--------|---------|
|                    | GRAMS  | %      | Actual      | Rougher | Final  | Actual                    | Rougher | Rougher       | Final | Gangue |         |
| F <sub>c</sub> - I | 243.5  | 27.5   | 66.0        |         | (66.0) | 18.15                     |         |               | 85.0  | (7.3)  | +77.7   |
| M - I              | 156.9  | 17.8   | 28.1        |         |        | 5.00                      |         |               |       |        |         |
| F - I              |        | (45.3) |             | (51.2)  |        |                           | (23.15) | 89.1          |       | (22.2) | +66.9   |
| S - I              | 481.0  | 54.7   | 5.9         | 5.9     | (5.9)  | 2.85                      | 2.85    | 10.9          | 15.0  |        |         |
| H - I              | 881.4  | 100.0  | (26.0)      | (26.0)  | (26.0) | (26.00)                   | 26.00   |               | 100.0 | 100.0  |         |

$$\text{RATIO OF CONCENTRATION: } K = \frac{66.0 - 5.9}{26.0 - 5.9} = 2.99 \quad \therefore \quad \omega = \frac{1}{2.99} = 33.5\%$$

REMARKS:

m = 77.5% Pb (cerussite)

$$E_m \text{ (rougher)} = 0.453 \left[ \frac{51.2}{26.0} - \frac{77.5 - 51.2}{77.5 - 26.0} \right] = 66.9\%$$

$$E_m \text{ (final)} = 0.335 \left[ \frac{66.0}{26.0} - \frac{77.5 - 66.0}{77.5 - 26.0} \right] = 77.7\%$$

$$\Delta \Phi \text{ (rougher)} = \frac{66.9\%}{14 \text{ min}} = +4.78 \text{ min}^{-1} \text{ %}$$

INVENTOR.

Alfonso Rizo-Patrón R.  
By: George, Innes, Watson +  
Churchill. 11115

June 18, 1963

A. RIZO-PATRÓN R

3,094,484

## PROCESS OF FROTH FLOTATION OF ORES

Filed Aug. 22, 1958

17 Sheets-Sheet 13

| TABLE NO. <u>II-E</u> |            |                          | Flotation <u>48</u>       |               |       | INVESTIGATION NO. <u>6 (3+4+5)</u>     |                        |
|-----------------------|------------|--------------------------|---------------------------|---------------|-------|----------------------------------------|------------------------|
|                       |            |                          | TEST NO. <u>48</u>        |               |       | PROBLEM NO. <u>Example 2</u>           |                        |
|                       |            |                          | CONDITIONS AND REAGENTS   |               |       | Cerro de Pasco Composite Ore: L10% Pb. |                        |
| POINT OF ADDITION     | CONDITIONS | REAGENTS POUNDS PER TON. |                           |               |       | OBSERVATIONS DURING TEST               |                        |
| TIME MINS.            | % SOLIDS   | PH                       | R-710<br>R-480<br>10% 6.6 | Nasil.<br>3.9 | R-710 | Ore<br>gr                              | H <sub>2</sub> O<br>cc |
| Grinding              | 30         | Nat                      | cc                        |               |       | 600                                    | 900                    |
|                       |            | 7.4                      |                           |               |       |                                        |                        |
| Conditioning          | 1          | 8.75                     | 60                        | 13 1/3        | 2.0   |                                        |                        |
| Rougher               | 10         | 8.75                     |                           |               |       |                                        |                        |
| Cleaner               | 5          | 8.50                     | No additions              |               |       |                                        |                        |
| Re-cleaner            | 4          |                          | "                         | "             |       |                                        |                        |

REMARKS: Test made in the San Isidro (Lima) laboratory of the "Cía. Minera Chancamino S.A."

Careful vanning and concentration of the coarse sediment of tailings gave 0.9 gr of a gray concentrate which was examined under a microscope (i) and re-united with S-48.

## METALLURGICAL RESULTS

| PRODUCT | WEIGHT   |           | Pb ASSAYS % |         | Pb CONTENT IN 100 PARTS/H |        | % DISTRIBUTIONS |       |        | Em     |        |
|---------|----------|-----------|-------------|---------|---------------------------|--------|-----------------|-------|--------|--------|--------|
|         | GRAMS    | %         | Actual      | Rougher | Final                     | Actual | Rougher         | Pb    | Pb     | Gangue |        |
| FRC-48  | 82.8     | 9.567     | 54.8        |         | (54.8)                    | 5.21   |                 |       | 65.0   | (3.95) | +61.05 |
| MRC-48  | 90.8     | 10.491    | 10.6        |         |                           | 1.12   |                 |       |        |        |        |
| Mc-48   | 230.5    | 26.632    | 5.4         |         |                           | 1.44   |                 |       |        |        |        |
| F-48    | (46.690) |           | (16.6)      |         |                           | (7.77) |                 | 79.3  | (42.1) |        | +37.2  |
| S-48    | 461.4    | 53.310    | 3.9         | 3.9     | (3.9)                     | 2.10   | 2.10            | 20.7  | 35.0   |        |        |
| H-48    | 865.5    | (600.009) |             | (9.87)  | (9.87)                    | (9.87) | (9.87)          | 100.0 | 100.0  |        |        |

$$\text{RATIO OF CONCENTRATION: } K = \frac{54.8 - 3.9}{9.87 - 3.9} = 8.5 \quad \therefore \quad w = \frac{1}{8.5} = 11.75\%$$

$$\text{REMARKS: * Assay of rougher} = \frac{7.77}{26.69} = 16.6\% \text{ Pb.}$$

$$Em \text{ (rougher)} = 0.4669 \left[ \frac{16.6}{9.87} - \frac{77.5 - 16.6}{77.5 - 9.87} \right] = +37.2\% \quad \Delta \Phi = +3.72 \text{ min}^{-1}\%$$

$$Em \text{ (final)} = 0.1175 \left[ \frac{54.8}{9.87} - \frac{77.5 - 54.8}{77.5 - 9.87} \right] = +61.05\%$$

(i) Examination under a binocular microscope of the vanned concentrate disclosed abundant limonite, hematite, some quartz, cerussite and anglesite, etc.. Also appreciable amount of sulphides such as enargite, chalcopyrite and pyrite; and perhaps some native silver too (a few silvery-white malleable particles). The proportion of oxidized lead minerals contained was minor.

Frc-48 under the microscope showed to be a practically pure concentrate of oxidized lead minerals.

## INVENTOR.

Alfonso Rizo-Patrón R.

BY *Berly, Townsend, Watson + Churchill* Atty's

June 18, 1963

A. RIZO-PATRÓN R

3,094,484

## PROCESS OF FROTH FLOTATION OF ORES

Filed Aug. 22, 1958

17 Sheets-Sheet 14

TABLE NO. II-FFlotation 84-85-86  
TEST NO. 92-95-96INVESTIGATION NO. 3  
PROBLEM NO. Example 2  
Cerro de Pasco Ore:  $\pm 11\% Pb$ .

| POINT OF ADDITION | CONDITIONS    |             |      | REAGENTS POUNDS PER TON.  |                                       |                         |               |       |                                                      | OBSERVATIONS DURING TEST |
|-------------------|---------------|-------------|------|---------------------------|---------------------------------------|-------------------------|---------------|-------|------------------------------------------------------|--------------------------|
|                   | TIME<br>MINS. | %<br>SOLIDS | PH   | Wg511. R-710<br>F3.22 10% | Na <sub>2</sub> CO <sub>3</sub><br>5% | NaNO <sub>3</sub><br>5% | Nas1.<br>3.22 | R-710 | Na <sub>2</sub> CO <sub>3</sub><br>NaNO <sub>3</sub> |                          |
| Grinding          | 20            | #60         | Nat. | drops                     | drops                                 | cc                      | cc            |       |                                                      |                          |
| Test 84           | 6             |             | 8.63 | 4                         | 17                                    | 1.25                    | —             | 8.1   | 1.61                                                 | 2.01                     |
| " 85              | 6             |             | 8.35 | 4                         | 17                                    | —                       | 1.25          | 8.6   | 1.73                                                 | 2.16                     |
| " 86              | 6             |             | 9.35 | —                         | 17                                    | 6.25                    | —             | —     | 1.81                                                 | 11.3                     |
| " 92              | 6             |             | 9.13 | —                         | 17                                    | 5                       | —             | —     | 1.66                                                 | 8.28                     |
| " 95              | 6             |             | 8.70 | 4                         | 17                                    | 0.6                     | —             | 10.3  | 2.06                                                 | 1.23                     |
| " 96              | 6             |             | 8.70 | 5                         | 17                                    | —                       | 1.25          | 12.9  | 2.07                                                 | 2.58                     |

REMARKS: 1 drop of Nas1.<sub>F</sub><sup>3.22</sup> = 2.5 lb/ton on 50 gr. ore basis.

## METALLURGICAL RESULTS

| PRODUCT | WEIGHT |      | % ASSAYS | $\Delta \Phi$<br>min <sup>-1</sup><br>% | Pb CONTENT IN 100 PARTS H | % DISTRIBUTIONS |        |         |       |
|---------|--------|------|----------|-----------------------------------------|---------------------------|-----------------|--------|---------|-------|
|         | GRAMS  | %    |          |                                         |                           | Pb              | Gangue | Em<br>% |       |
| F-84    | 18.8   | 30.4 | 26.6     | +8.73                                   | 8.10                      |                 |        | +52.4   |       |
| S-84    | 43.2   | 69.6 | 3.8      |                                         | 2.64                      |                 |        |         |       |
| H-84    | (62.0) |      |          |                                         | (10.74)                   |                 |        |         |       |
| F-85    | 17.6   | 30.4 | 26.7     | +8.58                                   | 8.11                      |                 |        | +51.6   |       |
| S-85    | 40.3   | 69.6 | 3.9      |                                         | 2.75                      |                 |        |         |       |
| H-85    | (57.9) |      |          |                                         | (10.86)                   |                 |        |         |       |
| F-86    | 29.9   | 54.0 | 16.0     | +3.81                                   | 8.65                      |                 |        | +22.95  |       |
| S-86    | 25.3   | 46.0 | 6.7      |                                         | 3.09                      |                 |        |         |       |
| H-86    | (55.2) |      |          |                                         | (11.74)                   |                 |        |         |       |
| F-92    | 30.1   | 49.8 | 14.7     | +3.72                                   | 7.31                      |                 |        | +22.4   |       |
| S-92    | 30.3   | 50.2 | 6.5      |                                         | 3.27                      |                 |        |         |       |
| H-92    | (60.4) |      |          |                                         | (10.58)                   |                 |        |         |       |
| F-95    | 14.2   | 29.2 | 29.5     | +9.12                                   | 8.6                       |                 | 76.0   | 21.1    | +54.9 |
| S-95    | 34.5   | 70.8 | 3.9      |                                         | 2.76                      |                 |        |         |       |
| H-95    | (48.7) |      |          |                                         | (11.36)                   |                 |        |         |       |
| F-96    | 10.1   | 20.8 | 28.4     | +6.5                                    | 5.9                       |                 |        |         | +39.0 |
| S-96    | 38.4   | 79.2 | 6.2      |                                         | 4.9                       |                 |        |         |       |
| H-96    | (48.5) |      |          |                                         | (10.8)                    |                 |        |         |       |

## RATIO OF CONCENTRATION:

REMARKS:  $\Delta \Phi = \frac{Em}{t}$  in min<sup>-1</sup> %

## INVENTOR.

Alfonso Rizo-Patrón R.

BY  
Byrd Townsend, Watson + Churchill  
Atty's.

June 18, 1963

A. RIZO-PATRÓN R

3,094,484

PROCESS OF FROTH FLOTATION OF ORES

Filed Aug. 22, 1958

17 Sheets-Sheet 15

FIG. 3



| Test No. | pH   | $\Delta\phi$ (1) | Test No. | pH   | $\Delta\phi$ | Test No. | pH   | $\Delta\phi$ | Test No. | pH   | $\Delta\phi$ |
|----------|------|------------------|----------|------|--------------|----------|------|--------------|----------|------|--------------|
| 51       | 7.01 | +0.32            | 58       | 8.40 | +6.10        | 65       | 8.45 | +8.96        | 72       | 8.59 | +7.88        |
| 52       | 7.40 | +0.46            | 59       | 8.90 | +1.3         | 66       | 8.80 | +0.7         | 73       | 8.49 | +7.35        |
| 53       | 8.03 | +1.80            | 60       | 8.35 | +4.39        | 67       | 7.16 | -0.15        | 74       | 8.95 | +8.20        |
| 54       | 8.45 | +2.17            | 61       | 8.65 | +9.45        | 68       | 7.95 | +4.00        | 78       | 8.79 | +8.85        |
| 55       | 8.76 | +0.14            | 62       | 9.00 | +8.40        | 69       | 8.75 | +8.36        |          |      |              |
| 56       | 7.52 | +0.60            | 63       | 8.37 | +8.35        | 70       | 9.35 | +2.83        |          |      |              |
| 57       | 7.93 | +4.82            | 64       | 8.67 | +0.4         | 71       | 8.52 | +8.67        |          |      |              |

Example 2

Oxidized lead ore  
from Cerro de Pasco

Conditions of Tests

Grind:

Dilution:  $\pm 60\%$  solids  
Ore weight: 900 grams  
Time: 10 minutes  
Fineness: 100% -48 mesh.

Flootation:

Dilution (Ps):  $\pm 25\%$  solids  
Weight of ore:  $1/16$  split portions  
Conditioning:  $\pm 1\frac{1}{2}$  minutes  
Time: as required.

Results

Equal differential floatability curves plotted.

$$\Delta\phi = \frac{w}{t} \left[ \frac{f}{h} - \frac{(m-f)}{(m-h)} \right]$$

$w$  = % weight of concentrate  
 $t$  = flotation time in minutes  
 $f$  = Pb grade of concentrate  
 $h$  = Pb grade of heads ( $\pm 11\%$ )  
 $m$  = Pb grade of cerussite (77.5%)

Predetermined Basic Conditions for Plant Operational Control:

Pulp density:  $d_p = \frac{d_o + 100}{P_s + d_o (100 - P_s)}$   
 $P_s = 25\%$   
 $d_o$  = specific gravity of the ore (experimental).

Reagents:  $\frac{NaSiI.}{R-710} = \frac{10.8}{2.25} = 4.8$

Resultant pH:  $\pm 8.85$  and "dp" (to be reached and maintained in the plant thru the controlled addition of the proportioned reagents).

INVENTOR.

Alfonso Rizo-Patrón R.  
BY: Beverly Ironman,  
Wilson + Churchill  
Atty's

June 18, 1963

A. RIZO-PATRÓN R

3,094,484

PROCESS OF FROTH FLOTATION OF ORES

Filed Aug. 22, 1958

17 Sheets-Sheet 16

FIG 4



SECTION A-A'

| Test No. | pH   | $\Delta\Phi$ (1) | Test No. | pH   | $\Delta\Phi$ |
|----------|------|------------------|----------|------|--------------|
| 99       | 8.23 | +1.87            | 108      | 8.68 | +5.92        |
| 100      | 8.13 | +7.10            | 109      | 9.00 | +2.35        |
| 101      | 8.40 | +6.90            | 110      | 7.80 | +3.85        |
| 102      | 8.25 | +2.06            | 111      | 8.60 | +9.15        |
| 103      | 7.12 | +1.66            | 112      | 9.35 | +0.53        |
| 104      | 9.15 | +0.18            | 115      | 8.60 | +4.24        |
| 105      | 7.25 | +3.80            |          |      |              |
| 106      | 7.68 | +6.62            |          |      |              |
| 107      | 8.05 | +7.49            |          |      |              |

(1):  $\Delta\Phi$  in % minutes<sup>-1</sup>.

Example 2

Low grade oxidized lead ore from Cerro de Pasco

Conditions of Tests

Grind:

1 batch of dry ore

Ore weight: 1,000 grams

Time: 15 minutes

Fineness: 100% -48 mesh

Flootation

Dilution: 50 gr. of ore in 250 cc. pulp

Weight of ore per test: 50 gr.

Conditioning: t 1 1/2 minutes

Time: as required by each test.

Results

Equal differential floatability curves plotted

$$\Delta\Phi = \frac{w}{t} \left[ \frac{f}{h} - \frac{(m-f)}{(m-h)} \right]$$

w = % weight of concentrate

t = flotation time in minutes

f = Pb grade of concentrate

h = Pb grade of heads (± 4.8%)

m = Pb grade of cerussite (77.5%)

Predetermined Basic Conditions for Plant Operational Control

$$\text{Pulp density: } dp = \frac{d_0 \times 100}{P_s + d_0(300 - P_s)}$$

$d_0$  = specific gravity of the ore (experimental)

$P_s$  = % solids in laboratory tests

$$\text{Reagents: } \frac{\text{NaSil.}}{R-710} = \frac{11}{2.8} = 3.93$$

Resultant pH: ± 8.60 and "dp" (to be reached and maintained in the plant through the controlled addition of the proportioned reagents and water).

INVENTOR

Alfonso Rizo-Patrón R.

BY: Buerly Townsend,  
Watson & Churchill,  
Atty's

June 18, 1963

A. RIZO-PATRÓN R

3,094,484

PROCESS OF FROTH FLOTATION OF ORES

Filed Aug. 22, 1958

17 Sheets-Sheet 17

FIG. 5



INVENTOR.

Alfonso Rizo-Patrón R.  
BY  
Bogoly, Townsend, Watson & Churchill  
Atty's.

# United States Patent Office

3,094,484

Patented June 18, 1963

1

3,094,484

PROCESS OF FROTH FLOTATION OF ORES  
Alfonso Rizo-Patrón R., A. de la Torre Gonzales 147,  
San Isidro, Lima, Peru  
Filed Aug. 22, 1958, Ser. No. 756,680  
15 Claims. (Cl. 209—166)

This invention relates to a metallurgical engineering improvement of the process of froth flotation of ores. It is particularly concerned with new methods for the determination of optimum metallurgical conditions and control of the same in the flotation of ores, that assure maximum practical efficiency during the industrial application of the process.

The invention is further related to the application of said improved methods in the flotation of oxidized ores amenable to treatment by means of a fatty acid or soap collector and an alkaline modifier.

It is furthermore specifically concerned with a practical application of flotation to the concentration of refractory oxidized lead ores with non-calcareous gangue, employing a silicated-soap reagent, prepared for, and used in the case of each individual ore, according to the mentioned new practical methods that control the maintenance of maximum flotation efficiency in the plant operation.

As is well known the flotation treatment of every ore requires the previous determination in the laboratory, by means of preliminary tests on a small scale, of the best conditions to carry out the process in practice, which involves choosing the most suitable reagents for the particular ore being treated, and proportioning the same properly. However, this is something much easier said than done as every ore needs special conditions for optimum results that are peculiar to its chemical and mineralogical composition; and every reagent must be specially proportioned in each case, to work at its best, not only in relation to its concentration in the solution of the pulp, and to the ore treated, but also in relation to other reagents used simultaneously. The chemical engineer's dream of designing generic flotation reagents capable of carrying out perfectly and under standard conditions the differential flotation of individual minerals of any ore in the presence of the complex associations and circumstances found in practice, has not materialized yet, and seems likely to remain a fond hope. Consequently, the laboratory testing work for each ore continues to be unavoidable.

The customary attempt to determine experimentally the optimum quantity of reagents has been a matter of cut and try. It has been considered an art, not a science. Experience and interest in one's work have counted heavily in this field.

This invention is particularly concerned with methods that will help make flotation testing work a more technically evaluated and precise undertaking and the flotation process in general more of a metallurgical engineering operation than an art, design of mechanical apparatus and/or prescription of formulas for chemical reagents, which by themselves cannot possibly assure the best metallurgical and economic solution for every type of ore, and yet have constituted almost all of the work done on the improvements of the previous art.

It has always been a difficult problem in metallurgical practice to determine the best among a series of experimental tests, or different operations; or the best compromise of several solutions, some better from the point of view of concentrate grade, and others with regard to recovery. The difficulty has stemmed principally from the lack of a just criterion, scientific and realistic at the same time, to measure the efficiency of a concentrating

2

operation, simultaneously from the two above-mentioned points of view. Under these circumstances it has been practically impossible to define accurately the best metallurgical conditions during the laboratory testing work, that would permit optimum results in the practice of flotation technology. The main problems involved in the laboratory testing work have been related to the optimum proportioning of reagents, and the control of other variables for the obtention of maximum results, consistent and industrially reproducible.

Furthermore, even supposing that the ideal metallurgical conditions for a given treatment have already been determined in the laboratory, it has always been more or less uncertain during the industrial operation of a plant, whether or not these ideal conditions were being reproduced in practice with their maximum efficiency. It often happens in flotation plants that the addition of many reagents is effected in an individual form, and generally the control of the multiple variables of the process is made separately for each one of them. Hence the joint effects can be evaluated only approximately, usually in an uncertain and defective way, precisely because of the lack of a realistic and scientific criterion with which to measure the metallurgical efficiency obtained. This situation has made it impossible to assure in any case that a given plant is operating with its best possible efficiency, even for the reagents combination that it is using, and for the machinery installed.

It is thus imperative in order to increase the efficiency of the flotation process in general not only to be able to assess properly the results of testing work or industrial operations, but also to evolve practical methods for maintaining the best predetermined conditions in the plant.

The present invention consists precisely of a series of integrated practical methods and physical steps based on and made possible by a new realistic assessment of the efficiency of a flotation operation, and designed with the object of teaching the men skilled in the practice of flotation technology how to determine practically the optimum conditions, metallurgical and economical, for the treatment of any ore, using any type or combination of reagents and flotation machinery; and subsequently how to apply said conditions on an industrial scale with their maximum efficiency; and how to control their constant maintenance in the operation of flotation plants. Consequently the methods of this invention constitute a new practical process, which comprises a series of coordinated steps, starting in the laboratory and ending with the production of re-cleaned concentrates in the flotation plant.

More specifically, a basis of the present invention has been the finding of simple formulas, derived from a logical definition of metallurgical objectives, that can be expressed in terms of the assays of the ore treated and of the products obtained in the flotation operation, and that measure for the first time with only one figure, expressed as percentage of the theoretically possible maximum efficiency, and by an index number that is also a function of time, in a scientific, just and realistic manner, the efficiency of a separation of the valuable elements from the gangue contained initially in the treated ore. These formulas take into account simultaneously the points of view of recovery, grade of the concentrate, ratio of concentration, nature of the ore treated and also the speed of the operation (flotation time).

The invention comprises also new methods to optimize the flotation process that are related to the practical achievement of its very objective of separating in the most efficient possible way, as defined by the above mentioned formulas, the valuable minerals from the gangue present in the ore treated during the actual plant operation.

The methods involved make use of chemical reagents, mechanical equipment, the new basic mathematical formulas discovered, chemical analyses, pH measuring and controlling electronic devices and specific process flow sheets as mere tools to achieve the intended ends of new, useful and improved results of the industrial flotation process.

The true metallurgical efficiency as herein disclosed is an adequate system of measurement for the degree of success achieved in a concentrating operation, whose objective is defined as the separation of the valuable mineral from the gangue (or of two groups of minerals or elements), initially contained in the ore treated. It is defined simply by the difference of the recoveries of the valuable mineral and of the gangue (or of two groups of minerals or elements) in the concentrate obtained in any concentrating operation.

The new kinetic concept of differential floatability which is a specific measure of flotation efficiency, takes into account the speed of the operation, and as herein disclosed, is defined as the difference of the mean specific flotation rates of the valuable mineral and of the gangue (or of two groups of minerals or elements) during the total flotation time interval; and it is given by the ratio of the metallurgical efficiency to the said flotation time. Its physical dimension is thus reciprocal time, and it is expressed in terms of percent over time.

The mathematical expressions of the formulas defining the above concepts in function of the products involved, assays of the same and of the ore treated, weight of the concentrate obtained, values of the heads and of the said involved products, and the flotation time, are as follows:

(A) Basic formulas:

$$(I) Em = RmF - RgF$$

$$(II) RmF = w \frac{f}{h}$$

$$(III) RgF = w \frac{(m-f)}{(m-h)}$$

$$(IV) Em = w \left[ \frac{f}{h} - \frac{(m-f)}{(m-h)} \right] = \frac{(h-s)}{(f-s)} \left[ \frac{f}{h} - \frac{(m-f)}{(m-h)} \right]$$

since

$$w = \frac{1}{K} \text{ and } K = \frac{f-s}{h-s}$$

$$(V) \Delta\Phi = Qm_{\text{overall}} - Qg_{\text{overall}}$$

$$(VI) Em = \Delta\Phi \cdot t \therefore \Delta\Phi = \frac{Em}{t}$$

(B) In the laboratory for rougher flotation batch tests:

$$(VII) \Delta\Phi = w \left[ \frac{f}{h} - \frac{(m-f)}{(m-h)} \right] \cdot \frac{1}{t} = \frac{(h-s)}{(f-s)} \left[ \frac{f}{h} - \frac{(m-f)}{(m-h)} \right] \frac{1}{t}$$

$$(VIII) \Delta\Phi_E = w \left[ \frac{\Sigma V_p}{\Sigma V_h} - \frac{(\Sigma V_m - \Sigma V_f)}{(\Sigma V_m - \Sigma V_h)} \right] \frac{1}{t_0}$$

and

$$\frac{1}{t_0} = \frac{\Sigma V_f \cdot F}{t}$$

(C) In the plant, for the continuous process:

$$(IX) P\Delta\Phi = \frac{(h-s)}{(f-s)} \left[ \frac{f_c}{h} - \frac{(m-f_c)}{(m-h)} \right] \frac{1}{T}$$

$$(X) P\Delta\Phi_E = \frac{(h'-s')}{(f'_c-s')} \left[ \frac{\Sigma V_{f_0}}{\Sigma V_h} - \frac{(\Sigma V_m - \Sigma V_{f_0})}{(\Sigma V_m - \Sigma V_h)} \right] \frac{1}{T_0}$$

and

$$\frac{1}{T_0} = \frac{\Sigma V_{f_0}}{T}$$

where:

$Em$  = Metallurgical efficiency (percent).

$RmF$  = Recovery of the valuable minerals in the froth concentrate F (float) (percent).

$RgF$  = Recovery of the gangue in the froth concentrate F (percent).

5  $w$  = Ratio of froth concentrate weight to weight of heads (weight of concentrate + weight of tailings).

$f$  = Grade (valuable element content) of the froth concentrate.

10  $h$  = Grade (valuable element content) of the heads, or calculated grade of heads as expressed in terms of the weights and assays of the products, froth concentrate and tailings, of the batch tests.

15  $m$  = Grade of the pure minerals being floated (weighted average assay of the pure minerals of the valuable element contained in the ore treated, that are being floated).

$s$  = Grade (valuable element content) of the tailings.

$K$  = Ratio of concentration.

20  $\Delta\Phi$  = Differential floatability (percent/time).

$Qm_{\text{overall}}$  = Mean specific flotation rate of the valuable mineral, for the total flotation time interval (reciprocal time).

25  $Qg_{\text{overall}}$  = Mean specific flotation rate of the gangue, for the flotation time interval (reciprocal time).

$t$  = Total flotation time interval of each laboratory rougher flotation batch test.

30  $\Delta\Phi_E$  = Differential floatability (percent monetary units per unit time) between all the valuable elements and the gangue, bulk or "economic differential floatability."

$\Sigma V_f$  = Sum of the values of the valuable elements contained in the rougher froth concentrate per ton of concentrate (monetary units).

35  $\Sigma V_h$  = Sum of the values of the valuable elements contained per ton of heads (monetary units).

$\Sigma V_m$  = Sum of the values of the valuable elements contained in one ton of the theoretically pure concentrate of the minerals of the valuable elements that are concentrated, present in the ore treated (monetary units).

40  $t_e$  = Average time required for the production of a quantity of concentrate with the value of one monetary unit by each laboratory rougher flotation batch test, during the respective total flotation time interval ( $t$ ).

45  $1/t_e$  = Reciprocal of said time, or production rate in terms of monetary units per unit time (economic capacity).

$F$  = Weight of froth concentrate produced by the laboratory rougher flotation batch tests.

50  $P\Delta\Phi$  = Plant differential floatability (in percent tons per hour).

$S$  = Grade of the final tailings (assay of the valuable element contained in the final tailing).

55  $f_c$  = Grade of the final cleaned froth concentrate obtained in the process (assay of the valuable element contained in the final cleaned froth concentrate).

$T$  = Time required for the production of one ton of final cleaned froth concentrate in the plant (in a fraction of an hour).

60  $1/T$  = Reciprocal of said time or production rate in tons of concentrate per hour (production capacity of plant).

$P\Delta\Phi_E$  = Plant differential floatability of all the valuable elements (percent monetary units per hour), "economic differential floatability in the plant."

65  $h'$  = Grade of the heads (assay of one of the valuable elements contained in the ore treated).

$S'$  = Grade of the final tailings (assay of the same valuable element contained in the final tailing).

70  $f'_c$  = Grade of the final cleaned froth concentrate obtained in the process (assay of the same valuable element contained in the final cleaned froth concentrate).

$\Sigma V_{f_0}$  = Sum of the values of the valuable elements contained in the final cleaned froth concentrate, per ton of concentrate (monetary units).

$1/T_e$ —Reciprocal of the time required for the production of a quantity of final cleaned froth concentrate with the value of one monetary unit in the plant (in a fraction of an hour), which is equivalent to the economic production rate of the plant.

As anyone familiar with flotation testing work will have noticed empirically the best conditions are generally associated with rapid floatability of the desired minerals. Consequently, when time is taken into consideration together with the metallurgical efficiency, that is to say, when the differential floatability as previously defined and measured, is taken as the criterion to assess flotation results, a complete evaluation of the true flotation efficiency is obtained, which sharpens dramatically the differences among the various relative results corresponding to different metallurgical conditions, permitting for the first time a precise determination of the best values of the controllable variables of the process.

The new formulas herein disclosed, permit for the first time the unequivocal determination of the best metallurgical conditions needed to produce optimum results in the practice of flotation technology, in function of the controllable variables of the process.

The values that could be determined as best for the controllable variables of the process through the evaluation of flotation results according to other yardsticks, previously available to the industry, such as the criteria of recovery, grade of concentrate, Gaudin's selectivity index, and, even the true metallurgical efficiency as herein disclosed, do not correspond exactly to the maximum values obtained by the differential floatability formulas. Consequently if as herewith sustained the latter give the only true assessment of the flotation process efficiency it follows that before the disclosures of the present invention it was materially impossible to determine accurately the optimum values of the controllable variables of the process in order to obtain the best possible results of the industrial operation.

The new formulas make it possible as a consequence of the true determination of optimum conditions, to evolve methods for an adequate technical control to insure their industrial scale application in flotation plants. Finally they permit a proper evaluation of the actual metallurgical results obtained in an industrial operation, in which way it is possible to compare said actual results with the optimum results obtainable, thus enabling management to have a close control of operational efficiency.

Thus the roughing operation should have as its true aim to achieve maximum differential floatability (maximum metallurgical efficiency in the minimum flotation time) and not simply to achieve a rough recovery of the bulk of the valuable minerals or a rough rejection of the bulk of the waste. Nothing is gained with a 100% recovery of the valuable mineral if simultaneously a 100% recovery of the gangue is effected; or with a 100% rejection of the gangue if simultaneously a 100% rejection of the valuable mineral is effected. In both these cases the flotation efficiency is zero, and yet the prior definition of roughing aims was vague enough to include both these extreme absurd possibilities.

Consequently the traditional practical expression of flotation operators that "the rougher flotation should be worked for recovery and the cleaner flotation should be worked for grade" is clearly incorrect. The roughing and cleaning operations of a flotation plant are not different processes with contradictory objectives, but rather two stages of the same process with the same objective. They should supplement each other, with the cleaning operation refining the results obtained in the roughing operations, and not un-doing them. Unfortunately the latter case was possible often enough with the previous vague understanding of the true aims of both operations.

Another basic finding of the present invention is that if

the maximum differential floatability conditions are established in the plant for the rougher operation, they will give place automatically to the greatest differential floatability conditions during the subsequent cleaning operations, which will accentuate therein, usually without the need of further reagent additions, the superiority of the rougher results, with respect to the results obtainable under other possible conditions, and thus assure the optimum economic and metallurgical final results for the complete process.

10 Therefore the rougher-scavenger operation should not be prolonged more than is absolutely necessary to produce results of maximum differential floatability. The metallurgical conditions necessary to achieve this purpose can be determined practically by the relative results of 15 batch laboratory rougher flotation tests performed with different amounts of reagents and under different conditions of the controllable variables.

The right flotation time will thus be a consequence of the use of proper reagent additions, under the correct 20 conditions to produce maximum rougher flotation efficiency.

The metallurgical conditions determined for laboratory rougher batch tests correspond to the initial conditions in said tests. Said initial conditions in the laboratory tests 25 correspond in turn to the steady-state conditions prevailing at the beginning of the rougher flotation circuit of the plant, and can thus be controlled best at the conditioning stage.

The continuous flotation operation in the plant can be 30 correlated to the operation of a single batch cell in the laboratory better than to the operation of a steady-state laboratory flotation cell. The approximation of test data obtainable from the ordinary laboratory batch cells is sufficiently accurate for all practical purposes notwithstanding the dilution necessary to counteract the shrinkage of pulp volume during the course of each laboratory batch test. Consequently this method of laboratory testing work has been proven most practicable for the objectives of the present invention.

40 The operation of a laboratory steady-state flotation cell may reproduce faithfully perhaps the operation of a single rougher cell of a plant. But the operation of a single laboratory batch rougher flotation cell reproduces more faithfully the operation of the total rougher string of cells 45 in the plant, since the operation of the first rougher cell of the plant can be correlated with the initial moment of the operation of the laboratory batch rougher cell, and the operation of the last scavenger cell of the plant circuit can be correlated to the last moments of the operation of the 50 laboratory cell. And of course a similar reasoning applies to the intermediate cells of the string of plant cells, and to the intermediate moments between initial and final conditions of the operation of the laboratory batch cell.

Hence in the present invention the steady-state initial 55 conditions corresponding to the maximum flotation efficiency determined in the laboratory with the rougher batch flotation tests, must be maintained in the conditioning stage at the plant. It is sustained here that the rest of the plant operation will give place to total conditions of 60 maximum efficiency as an inevitable consequence if this prerequisite is assured, which greatly facilitates the plant operational control.

The optimum proportioning in the feeding of reagents, for the best treatment of any ore, as well as the correct 65 determination of the other controllable variables of the process, become thus a real possibility for the first time through the above-defined metallurgical objectives.

The methods disclosed herein evolved from a practical application of this possibility to the treatment of refractory oxidized lead ores.

The novelty in its broad aspect of the methods embodying the present invention resides:

(a) In the invention or new formulas which define for the first time unequivocally the values of the controllable 75 variables of the process, namely, the grinding fineness,

pulp density, conditioning time, chemical collector, frother and modified reagents, and the resultant pH thereof, that produce conditions of maximum flotation efficiency, as measured by the difference of the mean rates of recoveries of the valuable minerals and of the gangue (or of two groups of minerals or metals) in the froth concentrate, during the total flotation time interval. This objective is the very essence of the flotation process, and yet had not been properly defined until now, or its true degree of success measured by the customary yard-sticks of the prior art.

(b) In the use of the resultant pH corresponding to the optimum values of the controllable variables, predetermined by the new formulas and laboratory methods that such as are described later in this specification as the controlling factor to reproduce and maintain in the plant said optimum values of the flotation variables. This is achieved by adding to the ore pulp in the plant the chemical collector, frother and modifier reagents in the predetermined optimum proportions, prior to the rougher flotation stage, but making the final adjustment for the feeding of the reagents in the conditioning stage, by reproducing therein the predetermined resultant pH, which is thus reached and kept in said conditioning stage, when the optimum amount of the combined reagents is being fed, thereby establishing and maintaining steady-state conditions corresponding to the variables required to produce maximum flotation efficiency in the rougher flotation stage.

(c) In the finding that if the maximum flotation efficiency conditions are established in the plant for the rougher operation, they will result automatically in the greatest flotation efficiency for the subsequent cleaning operations, and thus assure the optimum economic and metallurgical final results for the complete process. Therefore after establishing and maintaining in the conditioning stage the steady-state conditions corresponding to the variables predetermined to produce maximum flotation efficiency in the rougher flotation circuit, it is required that in the plant there is carried out a subsequent substantially open circuit continuous process, preventing re-circulation of pulp to the entrance of any flotation stage (which is contrary to usual prior art industrial flotation practice which involves closed circuit operation).

(d) In the discovery that the use of sodium silicate in the flotation of oxidized lead ores with non-calcareous gangue by means of a fatty-acid compound, in quantities far in excess of those heretofore used, produces much improved results as compared with the use of the customary quantities of sodium silicate employed by prior art methods. The improvement is such that the operation becomes industrially and economically feasible for the first time. The quantities of sodium silicate required vary with each ore, and can only be adequately determined and maintained in the plant by the methods summarized in the preceding paragraphs (a), (b) and (c); but are always larger than the quantities used by the prior art, and thus it is often found that the use of sodium silicate in quantities up to more than ten times greater than in the previous practice of the art produces the highest flotation efficiency and the best economic results, which only then become commercially profitable.

The invention will be better understood from the following detailed description when considered in connection with the accompanying drawings showing graphs and tables of laboratory tests and methods of evaluating same and wherein:

FIGS. 1 and 2 show graphs of equi-efficient curves plotted from laboratory tests on Pichita ores.

FIGS. 3 and 4 are analogous graphs from laboratory tests on Cerro de Pasco ores.

FIGS. 1a, 2a, 3a and 4a show graphs of sections taken along the planes of lines A—A<sup>1</sup> of FIGS. 1 to 4, respectively.

FIG. 5 shows the flow sheet of plant operations embodying the invention.

Tables IA to IF show actual conditions and results of some of the flotation tests on Pichita ores, that are plotted on FIGS. 1 and 2.

Tables IIA to IIF show actual conditions and results of some of the flotation tests on Cerro de Pasco ores, that are plotted on FIGS. 3 and 4.

The new methods that are of a strictly metallurgical engineering nature may be said to encompass the following steps:

#### 10 (1) IN THE LABORATORY

(a) Performing a series of batch rougher flotation tests in the usual way, but fixing all except two of the controllable chemical variables in each of the series of tests, carefully determining the resultant pH of each test.

15 (b) Making a series of tests for each of several grinding fineness (time of grinding in the laboratory), pulp density and conditioning time conditions.

20 (c) Plotting graphically the conditions corresponding to each test of every series in a system of Cartesian coordinates; fixing the scaled values of the two controllable variables of each series, according to the respective axes of abscissas and ordinates.

25 (d) Determining the differential floatability obtained in each test, calculated according to Formulas VII and VIII as required in each case and plotting them as the heights in a map of contour levels, for the corresponding points of the tests' conditions. The third spatial coordinate axis for the differential floatability is thus taken perpendicularly to the plane of the paper; in which way a three-dimensional coordinate system is established.

30 (e) Drawing the "contour levels" corresponding to the points of equal differential floatability by making the needed interpolations as is done in the topographic map with the data of heights of the surveyed points. A map of equal differential floatability curves is thus obtained for each series of tests that will have "hills" and "depressions." The curves of zero  $\Delta\Phi$  represent conditions of the studied variables that give place to a nil separation between the valuable mineral and the gangue. The positive curves express conditions corresponding to results that effect a concentration of the valuable mineral in the flotation froth. Negative curves express conditions corresponding to a concentration of the gangue in the froth.

35 In this form the chemical variables of the froth flotation process can be studied by pairs.

(f) The maximum (or minimum) points, "apex" of the "hills" (or "bottoms" of "depressions") represent of course the conditions of maximum separation efficiency between the valuable mineral and gangue of each tested ore; and the optimum conditions corresponding to each series of tests are thus precisely defined, and become apparent in the respective resulting "maps" at a glance.

40 (g) The optimum proportioning of reagents, giving place to maximum flotation efficiency, is thus unequivocally determined as well as the respective value of the resultant pH of the pulp for the adopted grinding conditions of each series of tests. It will be understood that grinding a given ore for various degrees of fineness is equivalent to changing the nature of the "heads" of the process, because the various minerals contained in the ore have different degrees of brittleness and thus give place to heads with different relative proportions of total surface area corresponding to each mineral species. Consequently the best chemical conditions for the same ore, under different grinding conditions, may and do vary substantially. From this fact follows the need of a different series of tests changing the chemical controllable variables for each condition of grinding adopted in an investigation, as well as for each of various pulp densities and conditioning times.

45 (h) Consequently the best grinding conditions can be determined by the relative results of each series of tests, through interpolations and repetitions of tests series for the inferred interpolated best grinding conditions. In this way by approximations, that can be carried out as far

as desired or as required by significant improvements, it is possible to determine experimentally the optimum grinding conditions for each ore, that produce the desired objective of maximum flotation efficiency in its concentration. This may be done through an experimental evaluation using the method described, better than through the usual mineralographic determinations and as demanded theoretically by the required liberation of values contained in the ore, because the best grinding conditions are determined on the basis of the achievement of the desired objective of maximum flotation efficiency directly.

(i) After the best grinding conditions to be used in the plant have been determined in the laboratory the mineralographic and other techniques can be used to define the resultant grinding fineness, and thus establish a reference basic control for repetition of said grinding conditions in the plant.

Hence in the laboratory testing work it will be possible to fix the best relative proportions of the reagents used, and the corresponding value of the resultant pH of the pulp, for a pulp density and degree of grinding for each ore that should reproduce the plant conditions. However in order to attain the best reproduction of said optimum results in the plant, the final flotation laboratory tests should be performed with the actual pulp ground in the plant after the desired degree of grinding fineness has been established in the plant operation.

## (2) IN THE PLANT

(a) Adding the reagents according to their optimum proportions predetermined in the laboratory, to the grinding section and/or conditioning tank ahead of each flotation circuit, and adjusting the final addition of the reagents solution only in said conditioning tank which may be controlled automatically, by regulating the addition of reagents until the resultant pH, determined in the laboratory as corresponding to the optimum conditions, is reproduced in the plant. This of course, will assure the addition of the total correct quantity of the reagents, properly proportioned, that is needed for the obtention of maximum flotation efficiency. In this form it is certain that the addition of reagents is performed constantly in the total quantity and proportions desired, during the industrial flotation operation, for reproduction in the plant of the maximum flotation efficiency reached in the laboratory.

It should be noted that in this method the pH is used not as an independent variable, but as the unique resultant of the addition of the reagents in the total amount and in the relative proportions that are most favorable as experimentally determined. This follows from the fact that there is only one resultant pH for the addition of a determined proportion of reagents to a pulp of given chemical, mineralogical, and physical (density and fineness of grind) nature and corresponding to a given contact time or reaction period.

The use that is made of the pH in the present invention is simply that of a dependent and resultant variable that corresponds to only one chemo-metallurgical climate for a given pulp, that is determined in the laboratory as explained before. Consequently the reproduction in the plant of said resultant pH (if the reagents are added in the predetermined form and proportions) guarantees automatically the exact reproduction on an industrial scale of said unique metallurgical climate corresponding to the maximum possible efficiency. This is to say that the pH is used in the new method as the most convenient medium of control, in order to assure the repetition in the plant of the maximum flotation efficiency conditions previously determined in the laboratory; because it is a variable that depends on, and results from, the reproduction of said maximum efficiency conditions in each case.

To make this concept clearer it should be remembered that a given pH can be obtained through many different reagent combinations. But the reverse does not apply, because for a given combination of reagents, in total

quantity and relative proportions defined with respect to each other and with respect to a given pulp, for the maximum flotation efficiency there is but one resultant pH, and only one. This is the basic principle that is utilized in the present practical process for the control of function of a flotation plant, working under predetermined conditions of maximum possible efficiency with the controllable variables adopted.

(b) Establishing a continuous substantially open circuit process operation, instead of the usual current practice that approaches a continuous closed-circuit flotation, with the middlings acting as the re-circulating load.

The current practice is described adequately in the latest book "Flotation," by Gaudin (1957), and involves the retreatment of tailings obtained in the cleaning operation, feeding them back together with the heads, or fresh pulp, to the entrance of the rougher circuit, where the froth concentrate of the scavenger circuit is also fed. Something similar is done with the tailing of the re-cleaner circuit that is added to the entrance of the cleaner circuit jointly with the froth concentrate of the rougher.

The practice would destroy to a considerable extent the metallurgical climate corresponding to the maximum rougher flotation efficiency conditions as determined in the laboratory and controlled according to this new method by the pH in the conditioner tanks ahead of the flotation circuits. For these reasons it is required during an industrial application of the new method not to return middlings at the entrance of any circuit, but rather to treat said middlings in independent circuits or to return them only near the exits of the principal circuits, in order that at least the major portion of the fresh pulp may react under the best possible conditions, without alteration of its most efficient metallurgical climate.

35 A qualitative circuit for the application of the new method is shown in FIG. 5, where the principles just mentioned are applied.

(c) Re-adjusting the pre-determined values of the controllable variables used for the basic rougher controlled conditions, as described under (a) and (b), making small changes in said values at time intervals sufficiently long to establish steady state conditions throughout the process, corresponding to each set of values of the controllable variables temporarily adopted.

(d) Assessing the corresponding effects in the process by measuring the rate of production of the final concentrate and by analyzing the heads, final tailings and said final cleaned froth concentrate produced in the overall process by each set of conditions, and evaluating the results according to one of the Formulas IX and X, as required in each case.

(e) Controlling the variations of the mentioned variables of the process and their steady state effects, by repeated readjustments according to the computation of the respective results obtained by said Formulas IX and X until the optimum values for the controllable variables producing maximum flotation efficiency are thus established in the plant.

The improved methods described in this specification were developed during the experimental work and evaluation of results in the case of the soap flotation of oxidized lead ores of the Pichita mine of Tarma, Peru; and later of oxidized lead ores from the deposit of Cerro de Pasco, Peru.

65 The application of the new method to these cases permitted favorable commercial solutions for the treatment of the ores of said deposits, which had been previously considered highly refractory for flotation treatment.

The best results obtained with the common fatty acids and sodium silicate reagents that were used, so far as I have been able to ascertain, correspond to proportions that had no precedent in the industry. Said novel proportioning of reagents, was responsible for the obtention of the necessary selectivity in the soap flotation of the oxidized lead ores treated, in order to reach commercial results.

Furthermore, the evaluation of the results obtained, by means of the system of equi-efficient curves that has been described, offered, as will be seen, proof that the optimum flotation efficiencies are obtained only within narrow limits of conditions, in such a fashion that if these precise conditions are not maintained in the plant without variation, according to the practical steps of control that are specified, disastrous results may be forthcoming, even with the use of the very same reagents that produce optimum conditions of flotation when they are duly proportioned.

This fact proves that it is not enough to have a good chemical prescription of flotation reagents, in order to obtain good results in a flotation plant. The proper metallurgical control and precise definition of conditions for each ore, such as provided by the methods of the present invention, are essential to obtain the desired optimum results.

The method hereinafter described involves the direct treatment by soap flotation of all the finely divided pulp of these ores. Thus, it does not require the aid of gravimetric concentration to be effective. Good results are obtained likewise without the need of desliming the ores prior to their flotation. In this way, the extraction of the contained values is effected from the total amount of the mine-run-ore, without the need of sacrificing the recovery of a large part of the floatable values usually contained in the slime fractions, that in these ores generally make up a big part of the original ore as it comes from the mine.

The method is applicable to oxidized lead ores, that contain a high proportion of iron, manganese, silica and aluminum oxides, even if they are clayish and slimy in nature; that is to say, precisely to those ores considered difficult or impossible to treat in the prior art. In this way the new method supplements the field of application of the flotation of oxidized lead ores by xanthates and aerofoams with previous sulphidization, that is applicable to ores with calcareous or just siliceous gangues.

The new method makes use of cheap reagents, the cheapest obtainable, but proportioned adequately to constitute a special "silicated-soap" reagent for each ore treated.

Thus the method makes use of a common higher fatty acid or any of its soaps, exemplified by oleic acid or red oil, fish oil fatty acids, tall oils, fatty acid amines, sulphonic acids, etc., that may be the cheapest obtainable, such as reagent 708 of American Cyanamid Company, or reagent 710, that is its sodium soap, as collector and frothing agent; and a common sodium silicate ("water glass"), or any of the soluble silicates, ortho, meta or sesqui-silicates, with a silica-alkali ratio normally lying between 0.50:1 and 3.98:1 (and that are generally marketed as water solutions of 18° to 67.5° Baumé), as the main modifying agent in the pulps.

That is to say that this new method depends for its success not on the use of new, complex and expensive chemical reagents, but on a combination efficiently proportioned, of known reagents, the simplest and cheapest obtainable, applied on an industrial scale according to the general metallurgical method described before, that permits an adequate control of their feeding in the plant, guaranteeing the best possible industrial results.

The improvement in the soap flotation process of oxidized lead ores that is embodied in the present invention, involves the use of sodium silicate as a modifying agent, in quantities that are considerably greater than the ones used in the prior art. This is economically possible due to the fact that sodium silicate is a very cheap reagent in relation to the cost of other usual flotation reagents, and due to the marked improvement that is obtained through this practice which precisely makes industrially and commercially feasible the flotation treatment of said ores.

On the other hand an excessive use of sodium silicate,

greater than required to obtain maximum efficiency, produces results of rapidly decreasing flotation efficiency, until conditions of no floatability are again obtained for the oxidized lead minerals.

5 In some of the ores treated by the present method it was verified, as can be seen in FIG. 1, and Table IA that for a given quantity of collector soap used, the employment of sodium silicate in quantities corresponding to the usual limits of previous metallurgical practice (test 10 25), gave place to flotation efficiencies even lower than for the use of the soap alone (test 24), without the addition of sodium silicate. The results for the flotation efficiency thus obtained were even negative.

However, using quantities of sodium silicate, of an 15 order of magnitude greater than the usual limitations of prior flotation practice, metallurgical efficiencies gradually higher were obtained until maximum values were reached with additions of sodium silicate in quantities several 20 times greater than the usual. Only then, a high degree of 25 selectivity and satisfactory economic solutions were obtained for the ores treated as will be evident from the graphs and tables. The addition of still greater quantities of sodium silicate produced by excess of reagent, decreasing results, until they were poor and even negative again.

These effects of the addition of sodium silicate during the soap flotation of oxidized lead minerals can be considered typical, although their intensity is variable according to the nature of each ore treated. The maximum 30 values correspond in all these cases to intermediate additions of sodium silicate, encompassed between added quantities that produce by defect or by excess very poor results.

The use of considerable quantities of sodium silicate 35 by the method involved in this invention permits also a good control of the froth produced during flotation by the soap collectors used, which is not easy to achieve otherwise.

Said large quantities of sodium silicate are variable for 40 each ore with optimum values comprised within rather narrow limits, and with the correct conditions determined according to the teachings of the new method in each case, very heavily laden and selective froths are obtained, of a silky aspect, that produce a very rapid flotation, and 45 with a very high degree of differential floatability between the oxidized lead minerals and the gangue, even in the presence of abundant quantity of iron and manganese oxides, as well as of clay and slimes.

For excessive quantities of sodium silicate, the froths 50 obtained become increasingly dry and brittle, and they lose gradually their frothing power until flotation becomes nil, with a scum-like aspect and little bubbles bursting almost as soon as formed. The selectivity is 55 also lost for these excessive quantities of sodium silicate, giving very poor results.

The feeding of "silicated-soap" should be effected to the grinding and/or conditioning circuit of a plant, simply through pipes and valves, as if it were water, which greatly facilitates control of the practical operation.

60 My experiments gave place to the following observations which might be helpful to an interested operator.

Flotation in the presence of slimes is carried out efficiently, with the obtention of froths that are heavily 65 mineralized, silky-looking, selective, not too bulky, with medium-sized bubbles, easy to handle, and that are readily cleaned and re-cleaned, yielding concentrates of very high grades.

At pH values below 9.5 moderate amounts of calcium 70 and magnesium salts, such as bicarbonates and sulfates, often found in mine or plant waters may be present in the water used for flotation without deleterious effects. In fact their influence seems to be beneficial, if anything, as tests performed in a mine laboratory, with the untreated water of the mine (of a pH=6.8) were con-

sistently better than tests performed in a city laboratory with water treated for city use (containing chlorine).

In general the use of fatty acids requires greater quantities of sodium silicate than the use of their soaps for the maximum respective results.

The total quantity required of liquid sodium silicate "as received" was found to be in all ores tested greater than in the prior art, and the best quantities were always much higher, in certain cases up to 50 or more pounds of silicate per ton of ore (see Table IF).

In general it may be stated that the amounts of sodium silicate needed in the process are greater than 6 pounds per ton.

The quantity of the collector soap or fatty acid needed for best results was never found to be less than 1.00 pound of collector reagent per ton of ore treated, in all the ores tested, which varied in grades from 4.5% to over 30% Pb; and values around 2 pounds of collector per ton of ore or slightly higher were usually found sufficient to reach the best results.

It is possible to use other alkalies to replace part of the sodium silicate modifying agent. With small amounts of alkalies such as soda ash (sodium carbonate), and sodium bicarbonate, in conjunction with a greater proportion of sodium silicate, good results may be obtained, that for rougher operations may be similar to the ones obtained with sodium silicate alone (see Table IIF).

In an industrial application of the process it is usually necessary to provide for ample cleaning and re-cleaning flotation cell facilities. The volume of the rougher float obtained in soap flotation of oxidized lead ores is usually much larger than is obtained in the flotation of sulphide ores, or with other types of collectors. Hence, the relative capacity of rougher, cleaner and re-cleaner cells necessary for the practice of this new method is generally different from the one required in other flotation processes. With this method a much greater relative capacity for the cleaner and re-cleaner cells is usually required.

In spite of the fact that the combined rougher float may be of relatively low grade, it is possible to obtain a high efficiency in the cleaning and re-cleaning operations, with the obtention of very high grade final concentrates, without the need of the addition of any other reagents, and generally carrying out the up-grading operations in less dense pulps, diluting them with water as necessary which is usually done in the launders while transferring the froth concentrates to the cleaning circuits.

In the operation of the pilot plant at the Pichita mine for example when treating an oxidized lead ore (assay 10.9% lead) with relatively high manganese content, which after grinding produced a pulp looking like a very dark brown mud, the rougher flotation gave place to concentrates of a light brown color (assay 26.1% lead), which by cleaning produced golden cream concentrates (assay 60.0% lead) and after re-cleaning a final concentrate was obtained (assay 65.0% lead) which was cream white in color; with tails assaying 4.9% lead. These results corresponded to proper flotation conditions for the ore treated. Then flotation in the rougher cells was quite rapid and with a loaded froth, not too voluminous in relation to its load. Flotation in the cleaner and re-cleaner cells was of highly increased selectivity.

It was in the above mentioned pilot plant operation that the best flow-sheet design to carry out this process was determined. The plant was originally installed according to the standard practice of returning middlings near the entrance of the fresh pulp to the rougher circuit. It became immediately apparent that the flotation conditions were completely spoiled in the rougher cells where middlings were returned. Bad conditions were also obtained in the cleaner cells where re-cleaner middlings were returned. It was thus proven in the pilot plant that the prior standard flow-sheet practice would be completely inoperative in practicing the present process and in fact the pilot plant capacity was reduced in the

preliminary test runs referred to in this example, to the capacity of the rougher flotation cells that were fed only fresh pulp with the addition of reagents controlled in the conditioned tank; and of the cleaner cells receiving only the fresh concentrates of the previous stage. It became then obvious that the proper flow-sheet for the practicing of this process involved the adoption of conditions approaching an open circuit continuous flotation operation, as previously described.

10 Laboratory procedures designed to achieve the purposes of the present invention and facilitate to the men skilled in the art, the application of its methods, will now be described. These experimental procedures were the ones utilized in connection with the testing work performed on the oxidized lead ores with non-calcareous gangue which served as a basis for the development of the new methods. Said procedures will illustrate a practical way of performing the testing work required in every case, according to the aims of the new invention. They however should not limit the novelty of the invention to the particular laboratory techniques involved.

15 In general the preliminary testing work may be performed on a very reduced scale, using small laboratory agitation type flotation machines with ore charges of around 50 grams per test. This practice permits covering a wide range of conditions, performing many tests in a relatively short time, and the easy handling, drying and weighing of the products obtained. Tests on this scale provide sufficiently accurate results for the rougher operations, and make possible to obtain comparative results, and all the data that is necessary for the evaluation of the corresponding differential floatabilities, according to the new formulas.

20 The grinding of the ore samples for these tests is made in batches of around 1 kilogram, or enough to provide the charges for a series of flotation tests under the same grinding conditions. In this way testing work is performed in several series of tests, corresponding to a grinding batch each and studying the variation of the chemical 25 controllable variables by pairs according to the general method described.

25 Conditions of each series of tests are maintained standardized for the other influencing variables of the process. The batch grinding for each group of tests should usually be performed with wet pulps, in the laboratory mills, at the highest pulp density permissible by the physical nature of every ore treated. Grinding time is controlled carefully, and the pulps are washed from the mill, using as little water as possible in the 30 operation. The wet pulp is then split into aliquot fractions used for the batch flotation tests. In this way practically uniform feed is assured for every test of the same series. Splitting requires some further dilution with water, which however is possible to maintain low, 35 with the obtention of charges with a pulp density above 25% solids by weight. The volume of each pulp for a batch test is adjusted in the flotation cell to a constant value for all tests. Then the addition of reagents is 40 controlled, and a standard conditioning period for each series of tests with slow agitation without air is allowed. The pH of the conditioned pulp is then measured for each test, after which flotation is allowed to take place while it lasts, and carefully controlling the corresponding period of time, through strong agitation with air. The froth 45 and tailing products obtained are dried, weighed, thoroughly mixed, sampled and assayed.

50 The data obtained permits the calculation of the assay and weight of heads for each test, and consequently the determination of the differential floatability obtained, according to the new formulas.

55 The data obtained from these small scale batch tests is tabulated in the normal way, with observations of the visual results of the tests, flotation conditions, character of froth and speed of the operation, etc.

60 With the data of conditions and the resultant differ-

sentential floatability of each test, a "map" corresponding to each series of tests is plotted according to the methods already described. Determination of the best flotation conditions, proportioning of reagents, and corresponding resultant pH is thus effected. The said best conditions, become apparent from the equal differential floatability curves on the maps and they usually do not in fact correspond to any one of the individual tests performed in the small scale series. They are then rather the result of obvious interpolations, or tendencies that are concretely defined in the said maps, which makes them a better method to determine the desired best conditions. The latter are then adopted for the performance of more quantitative tests on a larger scale (say 1000 grams of ore basis). For this purpose grinding as well as flotation is performed on a single batch charge. In this larger scale tests, grinding time and pulp density are fixed at their best predetermined values, and the addition of reagents is effected according to the proportions determined as best in the equal differential floatability curves maps. The resultant pH is then determined after the appropriate conditioning period, and the corresponding value is used for the later control of the industrial plant operation. The larger scale tests permit also the performing of cleaning and re-cleaning operations, retreating the froth of the rougher batch tests, either on the same laboratory flotation machine, or in smaller ones, according to the dilution desired for the operation, and the volume of the rougher float obtained in each case. The pH values are of course, controlled in these cleaning batch tests so that reference conditions for the plant may be obtained, correlating the batch laboratory tests to the corresponding open circuit cleaning and re-cleaning stages at the plant, for a proper control of dilution during these operations.

The problem of retreatment of the middlings obtained in the process may be studied independently of the one corresponding to the original ore. In some cases re-grinding may be necessary for further liberation of values contained in the concentrate or in the middlings. The special study of middlings re-treatment may of course be best made according to the new methods matter of this application, as if the middlings were a new ore.

In order to correlate plant conditions to the best results obtained in the laboratory using the resultant pH control method described, it is indispensable, as will be appreciated, to have a close control of the pulp density both in the laboratory and at the plant. It is thus required that the pulp density at the plant be the same as in the controlling laboratory final tests, in order that the values fixed for the variables to obtain best metallurgical conditions, may have any meaning during the plant operation.

Of course in the laboratory it is easy to produce any pulp density desired by weighing the ore and measuring the pulp volume. In the plant sometimes there are limitations imposed by factors dependent on the general flow-sheet, characteristics of the machinery used and physical conditions of every ore treated.

In order to facilitate the control of pulp density conditions during the application of the present process, the following formulas are proposed, because they are expressed in terms of variables that can be easily determined both in the laboratory and in the plant:

$$P_s = 100 \times \frac{d_o(d_p - 1)}{d_p(d_o - 1)} \text{ and } d_p = \frac{d_o \times 100}{P_s + d_o(100 - P_s)}$$

where:

$P_s$ =Percent solids in pulp (by weight).

$d_o$ =Specific gravity of ore treated (which can be determined accurately in the laboratory on a dried sample of the ground pulp of the ore), in metric units.

$d_p$ =Density of the flotation pulp (which is easily determined at the plant by weighing a measured volume of the said pulp), in metric units.

These formulas permit calculating readily the value of  $d_p$  for a given percentage of solids ( $P_s$ ) used in the laboratory tests (which in turn can be easily determined knowing  $d_o$ , the dry weight of the heads treated in the test, and the volume of the pulp in the flotation vessel used in the laboratory); or vice-versa. The value of  $d_p$  used to define in the laboratory the best metallurgical conditions and control factors for an application of the present process, must of course be faithfully reproduced in the plant.

The invention will be further illustrated, but it is not intended to be limited by the following specific examples of applications of its methods to oxidized lead ores with non-calcareous gangue from the two Peruvian mines "Pichita" and "Cerro de Pasco."

#### Example No. 1

The ores investigated were from the Pichita mine of Tarma, Peru. These ores are present in an oxidized surface formation containing the secondary enriched lead values, usually together with moderate to high percentages of iron and manganese oxides. Other constituents of these ores are quartz, silicates, aluminates (clay), etc.

These types of ores which are typical in the oxidized zone of lead ore deposits where strong weathering has taken place, are of an earthy, soft and slimy nature, and have previously been considered as not amenable to flotation treatment.

The use of xanthates and aero-floats with or without sulphidization was tried without success for the flotation treatment of these ores. Gravity concentration produced at best mediocre results, with low recoveries, and concentrate grades that were not sufficiently high, with the loss of all the fine particles of lead which are an important proportion of the values contained.

When customray xanthates flotation failed in these ores soap flotation was tried. Initial experiments showed it completely unselective, with results no better than with the use of xanthates. However, the accidental use of unintended large quantities of sodium silicate in a soap flotation test, produced momentarily very selective flotation conditions for the oxidized lead minerals. This led to a long and systematic study of conditions that eventually resulted in the development of the new methods.

The main testing work on the ores of the Pichita mine was made on two principal types of oxidized lead ores with non-calcareous gangue, containing respectively high or moderate proportions of manganese oxides. Early tests were performed mostly on the lower manganese content ores, containing from 8 to 20% lead. Favorable conditions were found for these ores for a sodium silicate-fatty acid ratio of about 15 to 1 by weight. A pilot plant was built based on these results and its operation was relatively successful from the start.

In early tests as well as in the operation of the pilot plant, reagent 708 of American Cyanamid Company was used as collector, with sodium silicate manufactured in Lima (silica-alkali ratio=3.9, 33° Bé.) as the only modifying agent. However, for later series of tests, the use of the soluble reagent 710, which is the corresponding soap was decided upon to facilitate measuring additions of the collector on the small scale tests, which were thus more accurately controlled. FIG. 1 shows the results obtained in the systematic series of tests for the high grade ore.

It will be appreciated that for additions of sodium silicate up to 10 pounds per ton in this ore the results obtained gave place to negative differential floatability; that is to say that the assays of the concentrates obtained were inferior to the assays of the original ore. All references of the prior art on the use of sodium silicate fall within this range. It will also be noted that for greater additions of sodium silicate this ore gave increasingly better results until for an addition of about 22 pounds per ton, corresponding to a fixed amount of soap used (3 pounds per ton) maximum differential floatability conditions were

obtained, which decreased for greater quantities of sodium silicate until the differential floatability became nil again for an addition of about 40 pounds per ton of sodium silicate. The best resultant pH for this ore was found to be about 9.15, which according to the teachings of the new method should be reached in the plant through the controlled addition of a silicated soap prepared by mixing 7.33 parts by weight of sodium silicate (of 3.9 silica to alkali ratio and 33° Baumé), and one part by weight of the American Cyanamid Company's fatty acid soap R-710. These results correspond to a 4-minute grinding time in the laboratory mill with more or less 60% solids, which is not necessarily the best grinding for optimum results. Consequently the results of FIG. 1 may probably be improved for other grinding conditions. However, these tests serve to illustrate clearly the methods of this invention.

The actual results of some of the tests included in FIG. 1 are given in Table IA, which will serve to illustrate the actual flotation conditions obtained in those tests in relation to the equal differential floatability curves graph of FIG. 1.

The differential floatability plotted correspond to the rougher flotation tests on a small scale. In order to illustrate the effect of cleaning operations in improving the obtainable flotation efficiency of the completed operation, reference is made to test 66 illustrated in Table IB, which after cleaning and re-cleaning produced a metallurgical efficiency of 50.6% in comparison to the 22.6% obtained in the rougher test.

FIG. 2 shows the results obtained with a 21% lead ore from the Pichita mine. Here the rougher small scale tests were made with dry grinding, and at a pulp density for flotation of 17.6% solids by weight. The specific gravity of this ground ore was experimentally determined to be 3.15. Consequently the pulp density to be maintained in the plant corresponding to said conditions was calculated to be 1.14, by applying the formula given before. The resultant pH obtained as most favorable was 8.90, when reached by the addition of a silicated soap made up by mixing a sodium silicate (of 30° Baumé with a silica-alkali ratio of 3.22, which had a specific gravity of 1.284), and the fatty acid soap R-710 in proportions corresponding to a ratio by weight of 17.7 to 1.

Table IC illustrates the conditions and the results of some of the tests included in the equal differential floatability curves of FIG. 2.

Table ID shows the results of tests 123 and 124 with the use of the soap R-710 and of the fatty acid 708, respectively under the good conditions determined for the use of soap 710 in FIG. 2. It will be noted that slightly better results were obtained by the use of the fatty acid R-708, and that in test 123 a better result was obtained with only a rougher operation ( $F_1$ ) than with a rougher and a scavenger operation ( $F_1+F_2$ ). The result of the rougher operation only was included in FIG. 2. Test 124 illustrates also the results obtainable through cleaning and re-cleaning operations under the given conditions.

It must be understood that the tests illustrated in this example are not exhaustive in defining the ultimate possibilities of the new method for the treatment of the ores tested. They have sufficed however to define the methods of the invention and illustrate the evaluation of flotation results with the equal differential floatability curves.

Test 131 illustrated in Table IE shows the results obtained with a sample corresponding to an ore similar to the composite sample used in tests of FIG. 2. The fatty acid R-708 was used and a grinding time of 6 minutes with a wet pulp at 45% solids by weight. The results show that for conditions similar to the ones determined in FIG. 2 very good results can be obtained at the plant, even though in this particular test the grinding was probably not sufficient for best liberation of values. The tailings obtained in this test were the lowest achieved with this type of ore. Said tailings were passed through a

laboratory Wilfley concentrating table and the corresponding results are also given in Table IE. The distribution of flotation and tabling middlings is also made in Table IE where the final results possible with the conditions of this test are equally shown. They prove that although there is still room for improvement, through new series of systematic tests at various grinding conditions, the results obtained are already sufficient to operate commercially, and they serve as well to illustrate a detailed use of methods of the new invention.

Table IF shows the results obtainable through finer grinding, even though the best variables had not been systematically evaluated for the corresponding conditions of the test illustrated. It will be seen that extremely high grade concentrates are possible when proper liberation of the lead values is obtained.

#### Example No. 2

The ores investigated were from the Cerro de Pasco mine of central Peru. They correspond to a large surface deposit of "pacos" (oxidized) ores that overlie the sulphide ore bodies of the Cerro de Pasco mine presently under exploitation.

The samples used in the testing work were as follows:

(a) Low grade ore (assay about 5% lead). Sample provided by the Cerro de Pasco Corporation laboratory at La Oroya in the month of July 1957. This sample was a composite of the formations outcropping in the "Matagente" open-cut. It had been labelled "unfloatable ore," and it contained cerussite as well as other oxidized lead minerals such as plumbojarosites. The most important gangue minerals appeared to be iron oxides, quartz and silicates; and it had a considerable amount of slimes although it was harder and not quite as clayish as the Pichita ores.

(b) A medium grade ore (assay about 11% lead), delivered at the Cerro de Pasco mine, and supposed to represent the average material of the ores of a stope under exploitation. The mineral composition of the ore was similar to the previous one, except that it had a greater proportion of cerussite.

(c) A high grade ore (assay about 26%), that was also delivered at the Cerro de Pasco mine, supposedly representing the higher grade ores that are exploited for direct shipment to the Oroya smelter. The mineralogical nature of this ore was also similar to the previous ones, but contained a higher proportion of cerussite.

Several preliminary tests applying the process already worked out for the Pichita ores, showed that the Cerro de Pasco ores responded readily to a similar treatment. However, it also became immediately apparent that the conditions required for these ores were quite different. Consequently a systematic series of tests and corresponding evaluation of results according to the methods of the new invention was made, using reagent 710 in the tests.

FIG. 3 illustrates the conditions and results obtained with the medium grade ore sample.

It will be seen that the best conditions of control for plant operation corresponded to the use of 2.25 pounds per ton of reagent 710 and 10.8 pounds per ton of sodium silicate (with a silica alkali ratio of 3.9, and 33° Baumé), that is to say a ratio by weight of modifier to collector of 4.8. When a silicated soap made up by the mixture of said reagents in the mentioned proportions is added to a pulp of similar fineness of grinding and density, as the pulp used in the tests, results of a metallurgical efficiency of about 56% and a differential floatability of around  $+11\% \text{ min.}^{-1}$  for the rougher operation may be expected. The resultant pH corresponding to said efficiency and conditions, may be estimated from the respective equal differential floatability curves map, that would be approximately 8.85, which is the value to be used for the plant control in order to obtain best results under the conditions prevailing in the series of test included in FIG. 3.

Table IIA shows the detailed conditions and results of some of the tests included in the equal differential floatability curves map of FIG. 3.

FIG. 4 illustrates the conditions and results obtained in the tests performed with the low grade ore sample of Cerro de Pasco. It will be appreciated that the best results correspond in this figure to the use of 2.8 pounds per ton of reagent 710, and 11 pounds per ton of sodium silicate with a silica alkali ratio of 3.22, and 30° Baumé. This proportion of reagents resulted in a sodium silicate to reagent 710 ratio by weight of  $\pm 3.93$ . The addition of this mixed reagent to a pulp similar to the one corresponding to the conditions of the tests of FIG. 4 will produce maximum differential floatability when a pH of about 8.6 is reached. And with these conditions the maximum results obtained in the series of tests of FIG. 4 would be a  $\Delta\Phi$  of about  $+10\% \text{ mins.}^{-1}$  for the rougher operation.

In order to illustrate further the superiority of the methods of this invention to evaluate flotation results over the old systems in a way that can be easily visualized, let us consider first tests 105 and 111 of Table IIB. The lead recoveries are respectively 51.0% and 54.7%, i.e., a very slight apparent difference. However the simultaneous recoveries of gangue were respectively 24.4% and 18.1%, which accentuates the superiority of test 111, giving for the resultant corresponding metallurgical efficiencies the values of  $+26.6\%$  and  $+36.6\%$ . However even this measure does not make full justice to the real superiority of test 111. This only becomes apparent when it is considered that the same flotation machinery, with a capacity to treat say 4,000 tons of ore per day, under the metallurgical conditions of test 105, which produced a metallurgical efficiency of  $+26.6\%$ , could treat 7,000 tons of the same ore per day, ground to the same fineness, under the metallurgical conditions of test 111 that produced a metallurgical efficiency of  $+36.6\%$ . The true measure of the relative merits of both results would thus be much more like the ratio of the respective differential floatabilities, which are 9.15 and 3.8. This means that test 111 is 2.4 times better than test 105, while the recoveries criterion showed almost equal results. The relative economic results will certainly be much more similar to the relative differential floatabilities than to the relative recoveries or metallurgical efficiencies.

From the point of view of recovery alone test 110 (recovery 60.5%;  $\Delta\Phi=3.85$ ) was better than test 111 (recovery 54.7%;  $\Delta\Phi=9.15$ ) and from the point of view of grade of the rougher concentrate, test 101 ( $Pb=15.4\%$ ;  $\Delta\Phi=6.9$ ) was also better than test 111 ( $Pb=13.2\%$ ). Considering only the metallurgical efficiency, test 107 ( $Em=37.4\%$ ;  $\Delta\Phi=7.48$ ) was in turn better than test 111 ( $Em=36.6\%$ ). The comparison of these results shows that the determination of the optimum value of the controllable variables was erratic and a real problem in the prior art. Only the differential floatability assessment of flotation results that takes into account metallurgical efficiency and flotation speed simultaneously gives an accurate and realistic measure of the overall efficiency of the flotation process and thus permits a precise and unequivocal determination of the values of the controllable variables assuring a true optimization of the industrial operation. Any other values of the controllable variables than called for by the differential floatability criteria would produce inferior technical and economic results in the process. This is the essence of the present invention and the basis of its practical importance to the flotation industry.

Table IIC shows the results and conditions of test 116 on a larger laboratory scale for the low grade ore of Cerro de Pasco. Unfortunately, the grinding conditions used were not the same as for the systematic tests of FIG. 4, and the pH adopted was according to test 107 and not 111, consequently peak efficiency conditions were not obtained in test 116. However, this test shows

that a relatively high grade concentrate (38.5% lead) can be obtained with the low grade plumbobajarites ores of Cerro de Pasco, even under conditions that are not the best.

Table IID shows the results of a test on 1000 grams of ore basis, performed with the high grade ore of the Cerro de Pasco deposit using the fatty acid R-708 as a collector and conditions inferred to work well from the results of the systematic testing done with the medium grade ores coming from the same section of the deposit and with the high grade oxidized lead Pichita ores that were studied in the maps of FIG. 1, FIG. 2 and FIG. 3. It will be appreciated that excellent flotation conditions were achieved for the high grade ore with the production of a high grade concentrate (assay 66% lead) with only one cleaning operation and with a total metallurgical efficiency of 79.5% after distribution of the middlings; which corresponded to a metallurgical efficiency for the rougher operation of 66.3%, that is to say better than was possible to obtain with the Pichita ores.

Table IIE shows the results and conditions of a laboratory test performed with a composite of the three ore samples of the Cerro de Pasco deposit that were available. Said composite was prepared by mixing the samples of the said three ores in the following approximate proportions by volume:

- (a) Low grade ore: 60%
- (b) Medium grade ore: 30%
- (c) High grade ore: 10%

The composite was crushed to minus  $\frac{1}{4}$ ", thoroughly mixed and a 900 gram sample was taken for a test on the large batch flotation cell of the laboratory. Conditions used were similar to the ones determined as optimum for the medium grade ore, as shown in FIG. 3, which may not have been the best for the composite. The results of this test show that satisfactory commercial results can be obtained with an average type of the oxidized lead ores from Cerro de Pasco.

Table IIF illustrates the results of some tests using soda ash (sodium carbonate) and sodium bicarbonate as modifying agents together with sodium silicate and alone. It will be seen that when the carbonate modifiers are used alone, without sodium silicate, abundant, persistent and rather unselective froths were obtained even at pH values over 9.00, which were rather similar to froths obtained by the use of soap alone without appropriate quantities of sodium silicate. However, mixtures of sodium silicate with lesser proportions of the carbonate alkalies produced good flotation results.

It must be understood however that all the tests given in this example were not exhaustive and more tests will be required to determine the best conditions, including optimum grinding fineness and pulp density with these ores.

The mentioned tests thus serve only as an illustration of the favorable reaction of the Cerro de Pasco ores to the present process, and as a further description of the methods embodied in this invention as applicable to the said ores.

It has thus been established by the above examples that oxidized lead ores with non-calcareous gangue of various grades and mineralogical compositions, and coming from different mines and various sections of the same, work well when treated according to the methods of this invention. It has been shown also that commercial results are obtainable through the new methods on the flotation concentration of these ores that had previously been considered "unfloatable."

Now it is well known that the very same reagents used to advantage for the flotation of oxidized lead ores, as specified herein, that is to say soaps or fatty acid collectors and sodium silicate or other alkaline modifiers, may be successfully applied under various conditions to the flota-

tion of many other metallic and non-metallic oxidized ores such as manganese oxides, tungsten ores (scheelite), uranium ores, iron ores, limestone ores, phosphate ores, tin ores (cassiterite), barite ores, oxidized copper ores, chromium ores, etc.

More specifically, in the treatment by flotation of any of the mentioned or other oxidized ores, using a sodium silicate or other alkaline modifiers and a fatty acid or soap collector, it is possible to design the most suitable modifier-collector mixture for each case, through exactly the same methods illustrated in FIGS. 1 to 4; as well as the resultant pH and other conditions necessary for plant control assuring maximum flotation efficiency.

The said mixed reagents may be added in the plant according to the methods of the present process, and a flow sheet design such as shown in FIG. 5 may be adopted for the most successful application of this invention to the treatment of any of the mentioned oxidized ores. Exactly the same improved methods and procedures involved in the process for the silicated-soap flotation of oxidized lead ores with non-calcareous gangue, would thus be applicable in those cases.

It will be furthermore apparent to the men skilled in the practice of flotation technology that the general methods described in this specification will permit the definition of the most efficient conditions for the froth flotation treatment of any ore, and the maintenance of the corresponding maximum flotation efficiency during the operation of industrial plants.

Summarizing it will be realized that the gradual better academic understanding of the scientific principles of flotation i.e., the fundamental physio-chemical nature of the phenomena involved in the complex systems dealt with by the froth flotation process of ores, which is provided by basic scientific research, can only lay the foundations to guide the experimental approach of applied research directed towards the design of specific solutions for the treatment of every ore. The chemical reagents, and the mechanical, electrical and electronic equipment provided for the purposes of the froth flotation process by the applied sciences of chemical, mechanical, electrical and electronic engineering respectively, constitute the basic tools at the disposal of the metallurgical engineering applied science, with which to work out the specific solutions needed for the best treatment of every ore. But said reagents or equipment cannot constitute by themselves a panacea of the problem because of its very nature and objectives, which are not chemical or mechanical, but metallurgical.

The flotation process (as well as other ore concentrating procedures) constitutes a typical process-metallurgical operation, that has the specific objective of obtaining maximum separation of the valuable from the gangue minerals (or in general of two groups of minerals or metals) contained in the treated ore in the minimum time and usually at the lowest possible cost, provided that the mentioned sought technical objective is efficiently achieved.

It is through practical coordinated methods based on the metallurgical engineering approach and evolved for maintaining in the plant the optimum values of the controllable variables of the process, pre-determined in the laboratory, and such as are involved in the methods just described, matter of this invention, that the froth flotation process may become gradually more of an applied science, or technology, than an art, as it is still considered.

It is furthermore through such engineering methods that the wasteful practice of many flotation operators to perform costly experiments during the operation of a flotation plant, may be checked by management and circumscribed to small variations of the best pre-determined conditions according to methods such as embodied in the present invention, to refine in the plant the peak conditions for optimum flotation efficiency. This of course becomes possible through the new formulas to evaluate the true flotation efficiency obtained during the plant operation,

from the data of the assays of products and production rate (economic capacity) that have been given for the first time in these specifications.

It will also be appreciated that the methods involved in this invention permit for the first time the accurate determination in the laboratory and in the plant of the true values of the controllable variables of the flotation process that actually produce optimum results; and thus they should help to improve the operating efficiency of every flotation plant. It is very unlikely that every plant is operating at its top possible efficiency, with solutions arrived at by the cut and try methods of the prior art, or by the overcomplicated and yet defective systems of assessment of flotation results previously available. It is thus most probable that the efficiency of every flotation plant is susceptible of some improvement in a greater or lesser degree, according to individual circumstances, by practicing the teachings of the present invention.

What I claim is:

1. The method to optimize the process of froth flotation of ores, which comprises pre-determining by a series of laboratory rougher flotation batch tests on the ores, the values of the controllable variables viz., fineness of grind, pulp density, chemical collector, frother and modifier reagents, conditioning time and the pH resulting from said variables that produce conditions of maximum differential floatability, as defined by the algebraic difference of the mean rates of recoveries of the valuable minerals and of the gangue in the froth concentrate during the total flotation time interval of the batch tests; varying the proportions of two chemical reagents in each series of tests for various grinding finenesses and for each of various fixed combinations of other reagents, pulp densities and conditioning times of the ground ores; measuring the resultant pH corresponding to each batch test of every series; expressing the conditions of the batch tests as functions of the pair of chemical reagents varied, as measured along the coordinate axes of a Cartesian system; noting at the plotted points the differential floatability of each test, drawing curves of equal differential floatability for the experimental results of each series of tests, the zero curves representing conditions of no separation of the valuable minerals from the gangue, positive curves representing conditions of concentration of the valuable minerals in the froth, and negative curves representing conditions of concentration of the gangue in the froth; taking from said equal-differential floatability curves the best relative proportion indicated by the respective coordinates of the pair of chemical reagents which produces the greatest absolute value, positive or negative, for the differential floatability in each series of tests, defining thus the conditions corresponding to the maximum differential floatability of all the series of tests, for the treatment of any ore in terms of the controllable variables of the process, and their resultant pH.

2. The method according to claim 1, which comprises weighing and analyzing for their grade (valuable element content) the products of each laboratory rougher flotation batch test, namely the froth concentrate and the tailings, and wherein the differential floatability is given in terms of the resulting weights and analyses and of the total flotation time interval of each of said batch tests, by the following expression:

$$\Delta\Phi = w \left[ \frac{f}{h} - \frac{(m-f)}{(m-h)} \right] \cdot \frac{1}{t} = \frac{(h-s)}{(f-s)} \left[ \frac{f}{h} - \frac{(m-f)}{(m-h)} \right] \frac{1}{t}$$

which is equivalent to:

$$\Delta\Phi = \frac{1}{t} [R_m F - R_g F]$$

i.e. to the algebraic difference of the recoveries of the valuable minerals and of the gangue in the froth concen-

trate obtained in each of the batch tests, divided by the corresponding total flotation time interval; and where:

$\Delta\Phi$ =differential floatability (percent/time)

$t$ =total flotation time interval of each laboratory rougher flotation batch test

$w$ =ratio of froth concentrate weight to weight of heads (weight of concentrate+weight of tailings),

$$w = \frac{w_F}{w_F + w_s}$$

$f$ =grade (valuable element content) of the froth concentrate

$h$ =grade (valuable element content) of the heads, or calculated grade of heads as expressed in terms of the weights and assays of the products, froth concentrate and tailings, of the batch tests,

$$h = \frac{w_F f + w_s s}{w_F + w_s}$$

$s$ =grade (valuable element content) of the tailings

$m$ =grade of the pure minerals being floated (weighted average assay of the pure minerals of the valuable element contained in the ore treated)

$R_m F$ =recovery of the valuable minerals in the froth concentrate,

$$= w \frac{f}{h}$$

$R_g F$ =recovery of the gangue in the froth concentrate,

$$= w \frac{(m - f)}{(m - h)}$$

3. The method according to claim 1, wherein the ore treated contains more than one valuable element, in which the differential floatability between all the valuable elements and the gangue is given by the following expression:

$$\Delta\Phi_E = w \left[ \frac{\Sigma V_f}{\Sigma V_h} - \frac{(\Sigma V_m - \Sigma V_f)}{(\Sigma V_m - \Sigma V_h)} \right] \frac{1}{t_e}$$

where:

$\Delta\Phi_E$ =differential floatability (percent monetary units per unit time) between all the valuable elements and the gangue, or "economic differential floatability"

$\Sigma V_f$ =sum of the values of the valuable elements contained in the rougher froth concentrate per ton of concentrate (monetary units)

$\Sigma V_h$ =sum of the values of the valuable elements contained per tons of heads (monetary units)

$\Sigma V_m$ =sum of the values of the valuable elements contained in one ton of the theoretically pure concentrate of the minerals of the valuable elements that are concentrated, present in the ore treated (monetary units)

$t_e$ =average time required for the production of a quantity of concentrate with the value of one monetary unit by each laboratory rougher flotation batch test, during the respective total flotation time interval ( $t$ ), given by

$$t_e = \frac{t}{(\Sigma V_f \cdot F)}$$

$1/t_e$ =reciprocal of said time, or production rate in terms of monetary units per unit time (economic capacity)

$F$ =weight of froth concentrate produced by the laboratory rougher flotation batch tests (in fractions of a ton).

4. The method according to claim 3, in which where a differential flotation operation with the obtention of more than one concentrate in more than one flotation stage for a complex ore is carried out, the differential floatability is given by the algebraic difference between the mean rates of recoveries of the valuable minerals that are being concentrated in each stage and of the group of other valuable minerals together with the gangue in the froth concentrate obtained in the same respective stage by each of the laboratory differential flotation rougher batch

tests, during the total flotation time intervals of said respective batch tests.

5. The method according to claim 1, which comprises forming in the plant a finely divided pulp of the ore, ground to the fineness and diluted to the pulp density predetermined to produce maximum differential floatability by the laboratory rougher flotation batch tests; conditioning said pulp by the controlled addition of the modifier, the collector and the frother reagents in the relative proportions and during the time also predetermined by the laboratory batch tests to produce maximum differential floatability; adding said reagents ahead of the rougher flotation circuit until the resultant pH corresponding to the proportion of total amount of reagents to ore pulp that produces maximum differential floatability as predetermined by the laboratory batch tests is reached and maintained in the conditioning stage of the plant; thereby establishing steady state conditions that reproduce continuously in the plant's operation the values of the controllable variables corresponding to the maximum differential floatability pre-determined for every ore, by the laboratory rougher flotation batch tests and the equi-differential floatability curves.

6. The method according to claim 5, wherein the froth flotation treatment of the ores comprises a continuous substantially open circuit process for the rougher, cleaner and re-cleaner flotation stages in the plant.

7. The method according to claim 6, wherein for establishing a continuous substantially open circuit process operation for the flotation of the ores, under rougher controlled conditions assuring maximum differential floatability, the middlings of the cleaner and re-cleaner circuits are returned near the exits of the rougher and cleaner circuits respectively.

8. The method according to claim 7, wherein the ores treated are ores of oxygen containing minerals, the chemical modifier contains at least one alkali and, each collector and frother is a fatty acid compound, which comprises forming a solution containing said modifier, and

40 said collector-frother mixed in their relative proportions pre-determined by the laboratory rougher flotation batch tests for every ore treated to produce maximum differential floatability; adding said mixed reagents solution to the ore pulp ahead of the rougher flotation circuit of the plant, making the final adjustment for the feeding of said reagents solution in the conditioning stage, by reproducing therein the density of the pulp and the resultant pH value corresponding to the relative proportion of total amount of reagents to ore pulp also pre-determined by the laboratory rougher flotation batch tests to produce maximum differential floatability; which pH is thus reached and maintained in said conditioning stage when said pre-determined proportion of the mixed reagents solution in relation to the ore pulp is being fed, thereby establishing and controlling during plant operation steady state conditions assuring the obtention of maximum differential floatability in the rougher flotation circuit of the plant.

9. The method according to claim 8, wherein the ores treated are oxidized lead ores with non-calcareous gangue, the modifier reagent is a soluble sodium silicate, and the collector-frother reagent is selected from the group of higher fatty acids, resin acids, fatty acid amines, sulfonic acids, mixtures thereof and their soluble soaps.

10. The method according to claim 9 in which the soluble sodium silicate used has a silica-alkali ratio lying between 0.50 and 3.98 and is in solution with a concentration between 18° and 67.5° Baumé.

11. The method according to claim 10 in which the total quantity of sodium silicate modifier used is greater than 6 pounds of sodium silicate solution "as received" per ton of ore.

12. The method according to claim 5 which comprises re-adjusting in the plant the pre-determined values of the controllable variables of the flotation process used for

the basic rougher controlled conditions, by making small changes in the proportions of the chemical modifier, collector and frother reagents for each of various ore feeding rates to the grinding circuit and respective classifier adjustments and for each of various pulp densities of the ores, at time intervals sufficiently long to establish steady state conditions throughout the process corresponding to the set of values of the controllable variables temporarily adopted, permitting the evaluation of the corresponding effects in the process by analyzing the heads, final tailings and final cleaned froth concentrate produced in the overall process by each set of conditions and by measuring the rate of production of said final concentrate (reciprocal of its flotation time); and controlling the variations of the mentioned variables and their steady state effects in the process by repeated readjustments and by computing the respective resultant plant differential floatabilities as given by the algebraic difference of the recoveries of the valuable minerals and of the gangue in the cleaned froth concentrate obtained as a final product of the process multiplied by its rate of production (capacity of plant); until the optimum values for the controllable variables producing maximum plant differential floatability are thus established; thereby precisely determining in each particular plant and maintaining for its operation, conditions that assure the obtention of optimum plant differential floatability in the overall industrial process.

13. The method according to claim 12, wherein the plant differential floatability is expressed and can be computed in terms of the analysis of heads, final tailings and final cleaned froth concentrate of the process and of the rate of production of said concentrate as follows:

$$P\Delta\Phi = \frac{h - S}{fc - S} \left[ \frac{fc}{h} - \frac{m - fc}{m - h} \right] \frac{1}{T}$$

where

$P\Delta\Phi$ =plant differential floatability (in percent tons per hour)

$h$ =grade of the heads (assay of the valuable element contained in the ore treated)

$S$ =grade of the final tailings (assay of the valuable element contained in the final tailing)

$T$ =time required for the production of one ton of final cleaned froth concentrate in the plant (in a fraction of an hour)

$\therefore 1/T$ =reciprocal of said time=production rate in tons of concentrate per hour (production capacity of plant)

$fc$ =grade of the final cleaned froth concentrate obtained in the process (assay of the valuable element contained in the final cleaned froth concentrate)

$m$ =grade of the pure minerals being floated (weighted average assay of the pure minerals of the valuable element contained in the ore treated).

14. The method according to claim 12, wherein the ore treated contains more than one valuable element, in which the plant differential floatability between all the valuable elements and the gangue is expressed as follows:

$$P\Delta\Phi_E = \frac{(h' - S')}{(f'c - S')} \left[ \frac{\Sigma V_{fe}}{\Sigma V_h} - \frac{(\Sigma V_m - \Sigma V_{fe})}{(\Sigma V_m - \Sigma V_h)} \right] \frac{1}{T_e}$$

$P\Delta\Phi_E$ =plant differential floatability of all valuable ele-

ments (percent monetary units per hour) or economic differential floatability in the plant

$h'$ =grade of the heads (assay of one of the valuable elements contained in the ore treated)

5  $S'$ =grade of the final tailings (assay of the same valuable element contained in the final tailing)

$f'_c$ =grade of the final cleaned froth concentrate obtained in the process (assay of the same valuable element contained in the final cleaned froth concentrate)

10  $\Sigma V_{fe}$ =sum of the values of the valuable elements contained in the final cleaned froth concentrate, per ton of concentrate (monetary units)

$\Sigma V_h$ =sum of the values of the valuable elements contained per ton of heads (monetary units)

15  $\Sigma V_m$ =sum of the values of the valuable elements contained in one ton of theoretically pure concentrate (monetary units)

1/  $T_e$ =reciprocal of time required for the production of a quantity of final cleaned froth concentrate with the value of one monetary unit in the plant (in a fraction of an hour) which is equivalent to the economic production rate of the plant.

15. The method according to claim 14, in which where 25 a differential flotation operation with the obtention of more than one concentrate in more than one flotation stage for a complex ore is carried out in the plant, the differential floatability for each stage of the process is given by the algebraic difference between the recoveries of the valuable minerals that are concentrated in each 30 differential stage and of the group of other valuable minerals together with the gangue in the final cleaned froth concentrate obtained in the same respective differential flotation stage of the plant, multiplied by the corresponding rate of production (reciprocal time) of the final concentrate in each differential flotation stage of the plant.

#### References Cited in the file of this patent

##### UNITED STATES PATENTS

- |    |           |         |       |               |
|----|-----------|---------|-------|---------------|
| 40 | 2,231,265 | Gaudin  | ----- | Feb. 11, 1941 |
|    | 2,286,374 | Ray     | ----- | June 16, 1942 |
|    | 2,703,646 | Schoeld | ----- | Mar. 8, 1955  |
|    | 2,857,051 | Noblitt | ----- | Oct. 21, 1958 |

##### OTHER REFERENCES

- Fahrenwald, "Batch Flotation Test," Engineering and Mining Journal, volume 146, Number 1, pages 74-76.
- Schuhmann, "Flotation Kinetics," Journal of Physical Chemistry, pages 891-902, volume 46, 1942.
- 50 Sollenberger, Trans. AIME, Mining Engineering, June 1958, pages 691-693.
- Arbiter, "Flotation Rates and Flotation Efficiency," Mining Engineering, pages 791-796, September 1951.
- 55 Duval, Revue de l'Industrie Minerale, 1949, pages 726-743.
- Taggart, A. F., "Handbook of Mineral Dressing," John Wiley and Sons, Incorporated, New York (1945), pages 19-174 to 19-187.
- 60 Transactions of American Institute of Mining and Metallurgical Engineers, volume 169 (1946), pages 448-465.